# EUROPEAN PATENT SPECIFICATION

(11) **EP 3 940 722 B1**
(45) Date of publication and mention of the grant of the patent: **08.05.2024**
(21) Application number: 20890034.0
(22) Date of filing: 07.07.2020
(51) Int. Cl.: H01F 1/057, H01F 41/02

(54) **NEODYMIUM-IRON-BORON MAGNET MATERIAL, RAW MATERIAL COMPOSITION, PREPARATION METHOD THEREFOR AND USE THEREOF**
NEODYM-EISEN-BOR-MAGNETMATERIAL, ROHSTOFFZUSAMMENSETZUNG, VERFAHREN ZU IHRER HERSTELLUNG UND IHRE VERWENDUNG
MATÉRIAU D'AIMANT NÉODYME-FER-BORE, COMPOSITION DE MATIÈRE PREMIÈRE, SON PROCÉDÉ DE PRÉPARATION ET SON UTILISATION

(30) Priority: 21.11.2019 CN 201911150975
(43) Date of publication of application: 19.01.2022
(73) Proprietor: Fujian Golden Dragon Rare-Earth Co., Ltd., Longyan City, Fujian Province 366300 (CN)
(72) Inventor: FU, Gang, Longyan, Fujian 366300 (CN); HUANG, Jiaying, Xiamen, Fujian 361000 (CN); HUANG, Jixiang, Longyan, Fujian 366300 (CN); QUAN, Qichen, Longyan, Fujian 366300 (CN)
(74) Representative: karo IP
(86) International application number: PCT/CN2020/100587
(87) International publication number: WO 2021/098224

(56) References cited:
- EP-B1- 0 536 421
- CN-A- 103 077 796
- CN-A- 103 366 918
- CN-A- 104 064 346
- CN-A- 105 513 737
- CN-A- 106 128 673
- CN-A- 110 828 089
- JP-A- 2013 225 533
- JP-A- 2018 056 334
- JP-A- 2019 169 542
- US-A1- 2007 137 733
- US-A1- 2014 366 687

## Description

### Technical Field

The present disclosure relates to a neodymium-iron-boron magnet material, a raw material composition and a preparation method therefor and a use thereof.

### Background

The neodymium-iron-boron (NdFeB) magnet material with Nd₂Fe₁₄B as the main component has high remanence (Br), coercivity and maximum energy product (BHmax) with great comprehensive magnetic properties, and is used in wind power generation, new energy vehicles, inverter household appliances and so on. The rare-earth component of the neodymium-iron-boron magnet material in the prior art is usually dominated by neodymium with only a small amount of praseodymium. Although there are few reports in the prior art that replacing a portion of neodymium with praseodymium can improve the performance of the magnet material, the improvement is limited and still not significant. On the other hand, the neodymium-iron-boron magnet material with good coercivity and remanence properties in the prior art also need to rely on the addition of large amounts of heavy rare earth elements and the cost is relatively expensive.
EP 0 536 421 B1 discloses a method of producing a rare earth permanent magnet, wherein a platelike magnet material obtained by casting and hot working is formed in an accurate shape by hot bending.

### Content of the present invention

The technical problem to be solved in the present disclosure is for overcoming the defect that the coercivity and remanence of the magnet material cannot be significantly improved after the neodymium is replaced with the praseodymium partially in the neodymium-iron-boron magnet material in the prior art. A neodymium-iron-boron magnet material, a raw material composition and a preparation method therefor and a use thereof are provided. The content of praseodymium and copper in the neodymium-iron-boron magnet material of the present invention are increased at the same time, which can overcome the defect in the prior art in that the coercivity of the neodymium-iron-boron magnet material cannot be significantly improved when the content of praseodymium or copper is increased alone, and the remanence and coercivity of the obtained neodymium-iron-boron magnet material are both high.

At present, it is generally believed in the prior art that adding a small amount of copper to the neodymium-iron-boron magnet material can increase wettability. However, the inventors found through extensive experiments that after mating the specific content of praseodymium with the specific content of copper, non-magnetic phases such as RECu₂, RECu and RE₆Fe₁₃Cu appeared, wherein RE refers to neodymium and praseodymium elements, and the appearance of these non-magnetic phases effectively isolates the magnetic coupling between the crystal grains, and also improves the clarity of grain boundaries and optimizes the grain boundary phases, so that the performance of the neodymium-iron-boron magnet material can be further improved.

The present disclosure solves the above-mentioned technical problems through the following technical solutions:

The present disclosure provides a raw material composition of neodymium-iron-boron magnet material, wherein, the raw material composition of neodymium-iron-boron magnet material comprises the following components by mass percentage:
29.5-32% of R', R' is a rare earth element and includes Pr and Nd; wherein, Pr ≥17.15%;
Cu > 0.35%;
0.9-1.2% of B;
64-69.2% of Fe, the percentage refers to the mass percentage relative to the total mass of the raw material composition of neodymium-iron-boron magnet material.

In the present disclosure, the content of Pr is preferably 17.15-26%, for example 17.15%, 18.15%, 19.15%, 20.15%, 20.85%, 21.15%, 22.15%, 23.15%, 24.15%, 25.15% or 26%, the percentage refers to the mass percentage relative to the total mass of the raw material composition of neodymium-iron-boron magnet material.

In the present disclosure, the content of Nd is preferably 15% or less, more preferably 4-13%, for example 4%, 5.85%, 6.85%, 7.85%, 8.85%, 9.85%, 10.65%, 10.85%, 11.35%, 12.35% or 12.85%, the percentage refers to the mass percentage relative to the total mass of the raw material composition of neodymium-iron-boron magnet material.

In the present disclosure, the content of R' is for example 29.5%, 30%, 30.5%, 31%, 31.5% or 32%, the percentage refers to the mass percentage relative to the total mass of the raw material composition of neodymium-iron-boron magnet material.

In the present disclosure, preferably, R' further comprises other rare earth elements besides Pr and Nd, for example Y.

In the present disclosure, preferably, R' further comprises RH, RH is heavy rare earth element, the kind of RH preferably comprises one or more of Dy, Tb and Ho, more preferably Dy and/or Tb.

Wherein, the mass ratio of RH and R' is preferably less than 0.253, more preferably 0-0.07, for example 0, 1/32, 2/32, 2/31, 1.5/32, 2/32 or 1.5/31.

Wherein, the content of RH is preferably 1-2.5%, for example 1%, 1.5% or 2%, the percentage refers to the mass percentage relative to the total mass of the raw material composition of neodymium-iron-boron magnet material.

When RH comprises Tb, the content of Tb is preferably 0.5-2%, for example 0.7%, 0.8%, 0.9%, 1%, 1.5%, 1.8%, 1.9% or 2%, the percentage refers to the mass percentage relative to the total mass of the raw material composition of neodymium-iron-boron magnet material.

When RH comprises Dy, the content of Dy is preferably 1% or less, more preferably 0.3% or less, for example 0.1%, 0.2% or 0.3%, the percentage refers to the mass percentage relative to the total mass of the raw material composition of neodymium-iron-boron magnet material.

When RH comprises Ho, the content of Ho can be the conventional content in the field, for example 0.8-2%, preferably 1%, the percentage refers to the mass percentage relative to the total mass of the raw material composition of neodymium-iron-boron magnet material.

In the present disclosure, the content of Cu is preferably 0.35-1.3%, for example 0.35%, 0.4%, 0.45%, 0.5%, 0.6%, 0.65%, 0.7%, 0.8%, 0.85%, 0.9%, 0.95%, 1%, 1.05%, 1.1% or 1.2%, the percentage refers to the mass percentage relative to the total mass of the raw material composition of neodymium-iron-boron magnet material.

In the present disclosure, the content of B is preferably 0.95-1.2%, for example 0.985%, 1%, 1.1% or 1.2%, the percentage refers to the mass percentage relative to the total mass of the raw material composition of neodymium-iron-boron magnet material.

In the present disclosure, the content of Fe is preferably 64.8-69.2%, for example 64.914%, 64.965%, 65.065%, 65.085%, 65.135%, 65.365%, 65.405%, 65.485%, 65.54%, 65.615%, 65.665%, 65.715%, 65.815%, 65.865%, 65.915%, 66.015%, 66.035%, 66.045%, 66.215%, 66.23%, 66.265%, 66.315%, 66.465%, 66.445%, 66.545%, 66.615%, 66.715%, 66.815%, 66.865%, 67.145%, 67.165%, 67.415%, 67.615%, 67.915%, 68.015%, 68.295%, 68.565% or 69.165%, the percentage refers to the mass percentage relative to the total mass of the raw material composition of neodymium-iron-boron magnet material.

In the present disclosure, preferably, the raw material composition of neodymium-iron-boron magnet material further comprises Al.

Wherein, the content of Al is preferably 3% or less, more preferably 0.5% or less, for example 0.02%, 0.03%, 0.1%, 0.2%, 0.25%, 0.3%, 0.4%, 0.45%, 0.46% or 0.48%, the percentage refers to the mass percentage relative to the total mass of the raw material composition of neodymium-iron-boron magnet material.

In the present disclosure, preferably, the raw material composition of neodymium-iron-boron magnet material further comprises Ga.

Wherein, the content of Ga is preferably 1% or less, more preferably 0.05-0.6%, for example 0.1%, 0.15%, 0.18%, 0.2%, 0.24%, 0.25%, 0.3%, 0.4% or 0.5%, the percentage refers to the mass percentage relative to the total mass of the raw material composition of neodymium-iron-boron magnet material.

In the present disclosure, preferably, the raw material composition of neodymium-iron-boron magnet material further comprises Zr.

Wherein, the content of Zr is preferably 0.3% or less, for example 0.1%, 0.2%, 0.22%, 0.25%, 0.26%, 0.27%, 0.28%, 0.29% or 0.3%, more preferably 0.25-0.3%, the percentage refers to the mass percentage relative to the total mass of the raw material composition of neodymium-iron-boron magnet material.

In the present disclosure, preferably, the raw material composition of neodymium-iron-boron magnet material further comprises Co.

Wherein, the content of Co is preferably 0.2-1.5%, for example 0.2% or 1%, the percentage refers to the mass percentage relative to the total mass of the raw material composition of neodymium-iron-boron magnet material.

In the present disclosure, preferably, the raw material composition of neodymium-iron-boron magnet material can further comprise other conventional elements in the field, for example one or more of Zn, Ag, In, Sn, V, Cr, Mo, Ta, Hf and W.

Wherein, the content of Zn can be a conventional content in the field, preferably 0.1% or less, more preferably 0.04-0.08%, for example 0.04%, 0.05% or 0.08%, the percentage refers to the mass percentage relative to the total mass of the raw material composition of neodymium-iron-boron magnet material.

Wherein, the content of Mo can be a conventional content in the field, preferably 0.1% or less, more preferably 0.01-0.08%, for example 0.04%, 0.05% or 0.08%, the percentage refers to the mass percentage relative to the total mass of the raw material composition of neodymium-iron-boron magnet material.

In the present disclosure, the raw material composition of neodymium-iron-boron magnet material preferably comprises the following components by mass percentage: 29.5-32% of R', R' is a rare earth element and includes Pr and Nd; wherein, Pr ≥17.15%; Cu ≥0.35%; Al≤0.5%; 0.9-1.2% of B; 64-69.2% of Fe; more preferably, the content of Pr is 17.15-26%; more preferably, the content of Cu is preferably 0.35-1.2%; more preferably, R' further comprises RH, RH is a heavy rare earth element, the content of the heavy rare earth element is preferably 1-2.5%, the percentage refers to the mass percentage relative to the total mass of the raw material composition of neodymium-iron-boron magnet material.

In the present disclosure, the raw material composition of neodymium-iron-boron magnet material preferably comprises the following components by mass percentage: 29.5-32% of R', R' is a rare earth element and includes Pr and Nd; wherein, Pr ≥17.15%; Cu ≥0.35%; 0.25-0.3% of Zr; 0.9-1.2% of B; 64-68% of Fe; more preferably, the content of Pr is 17.15-26%; more preferably, the content of Cu is preferably 0.35-1.2%; more preferably, R' further comprises RH, RH is a heavy rare earth element, the content of the heavy rare earth element is preferably 1-2.5%, the percentage refers to the mass percentage relative to the total mass of the raw material composition of neodymium-iron-boron magnet material.

In the present disclosure, the raw material composition of neodymium-iron-boron magnet material preferably comprises the following components by mass percentage: 29.5-32% of R', R' is a rare earth element and includes Pr and Nd; wherein, Pr ≥17.15%; Cu ≥0.35%; Al≤0.5%; 0.25-0.3% of Zr; 0.9-1.2% of B; 64-69.2% of Fe; more preferably, the content of Pr is 17.15-26%; more preferably, the content of Cu is preferably 0.35-1.2%; more preferably, R' further comprises RH, RH is a heavy rare earth element, the content of the heavy rare earth element is preferably 1-2.5%; the kind of RH preferably comprises Dy and/or Tb, wherein, the content of Tb is preferably 0.5-2%, the content of Dy is preferably 1% or less; the percentage refers to the mass percentage relative to the total mass of the raw material composition of neodymium-iron-boron magnet material.

In the present disclosure, the raw material composition of neodymium-iron-boron magnet material preferably comprises the following components by mass percentage: 29.5-32% of R', R' is a rare earth element and includes Pr and Nd; wherein, Pr ≥17.15%; Cu ≥0.35%; Ga≤0.42%; 0.9-1.2% of B; 64-69.2% of Fe; more preferably, the content of Pr is 17.15-26%; more preferably, the content of Cu is preferably 0.35-1.3%; more preferably, R' further comprises RH, RH is a heavy rare earth element, the content of the heavy rare earth element is preferably 1-2.5%, the percentage refers to the mass percentage relative to the total mass of the raw material composition of neodymium-iron-boron magnet material.

In the present disclosure, the raw material composition of neodymium-iron-boron magnet material comprises the following components by mass percentage: 29.5-32% of R', R' is a rare earth element and includes Pr and Nd; wherein, Pr ≥17.15%; Cu ≥0.35%; Al≤0.5%; Ga≤0.42%; 0.9-1.2% of B; 64-69.2% of Fe; more preferably, the content of Pr is 17.15-26%; more preferably, the content of Cu is 0.35-1.3%; more preferably, R' further comprises RH, RH is a heavy rare earth element, the content of the heavy rare earth element is preferably 1-2.5%, the percentage refers to the mass percentage relative to the total mass of the raw material composition of neodymium-iron-boron magnet material.

In the present disclosure, the raw material composition of neodymium-iron-boron magnet material preferably comprises the following components by mass percentage: 29.5-32% of R', R' is a rare earth element and includes Pr and Nd; wherein, Pr ≥17.15%; Cu ≥0.35%; Ga≤0.42%;0.25-0.3% of Zr; 0.9-1.2% of B; 64-69.2% of Fe; more preferably, the content of Pr is 17.15-26%; more preferably, the content of Cu is 0.35-1.3%; more preferably, R' further comprises RH, RH is a heavy rare earth element, the content of the heavy rare earth element is preferably 1-2.5%, the percentage refers to the mass percentage relative to the total mass of the raw material composition of neodymium-iron-boron magnet material.

In the present disclosure, the raw material composition of neodymium-iron-boron magnet material preferably comprises the following components by mass percentage: 29.5-32% of R', R' is a rare earth element and includes Pr and Nd; wherein, Pr >_17.15%; Cu >_0.35%; Al≤0.5%; Ga≤0.42%; 0.25-0.3% of Zr; 0.9-1.2% of B; 64-69.2% of Fe; more preferably, the content of Pr is 17.15-26%; more preferably, the content of Cu is preferably 0.35-1.2%, more preferably, R' further comprises RH, RH is a heavy rare earth element, the content of the heavy rare earth element is preferably 1-2.5%; the kind of RH preferably comprises Dy and/or Tb, wherein, the content of Tb is preferably 0.5-2%, the content of Dy is preferably 1% or less; the percentage refers to the mass percentage relative to the total mass of the raw material composition of neodymium-iron-boron magnet material.

In the present disclosure, the percentage refers to the mass percentage of each component relative to the total mass of the raw material composition of neodymium-iron-boron magnet material.

The present disclosure further provides a preparation method for neodymium-iron-boron magnet material, which employs the raw material composition of neodymium-iron-boron magnet material mentioned above to prepare.

In the present disclosure, the preparation method preferably comprises the following steps: the molten liquid of the raw material composition of neodymium-iron-boron magnet material is subjected to melting and casting, hydrogen decrepitation, forming, sintering and ageing treatment.

In the present disclosure, the molten liquid of the raw material composition of neodymium-iron-boron magnet material can be prepared by the conventional method in the field, for example: melting in a high frequency vacuum induction melting furnace. The vacuum degree of the melting furnace can be 5×10⁻² Pa. The temperature of the melting can be 1500°C or less.

In the present disclosure, the operations and conditions of casting can be conventional in the field, for example, in Ar atmosphere (for example in Ar atmosphere of 5.5×10⁴Pa), cooling at 10² °C/sec-10⁴ °C/sec.

In the present disclosure, the operations and conditions of hydrogen decrepitation can be conventional in the field. For example, being subject to hydrogen absorption, dehydrogenation and cooling treatment.

Wherein, the hydrogen absorption can be carried out at the pressure of 0.15 Mpa.

Wherein, the dehydrogenation can be carried out under the condition of heating while evacuating.

In the present disclosure, the conventional pulverization in the field can be carried out after hydrogen decrepitation. The pulverization process can be conventional in the field, for example jet mill pulverization. The jet mill pulverization is preferably carried out in nitrogen atmosphere with 150ppm or less of oxidizing gas. The oxidizing gas refers to the content of oxygen or moisture. The pressure of the pulverization chamber of jet mill pulverization is preferably 0.38 Mpa; the time of the jet mill pulverization is preferably 3h.

Wherein, after the pulverization, lubricants can be added to the powder by the conventional method in the field, for example zinc stearate. The amount of lubricant added can be 0.10-0.15% of the weight of the mixed powder, for example 0.12%.

In the present disclosure, the operations and conditions of the forming can be conventional in the field, for example magnetic field forming method or hot press and hot deformation method.

In the present disclosure, the operations and conditions of the sintering can be conventional in the field. For example, preheating, sintering and cooling in vacuum (for example in vacuum of 5×10⁻³ Pa).

Wherein, the temperature of the preheating is usually 300-600°C. The time of the preheating is usually 1-2h. The preheating is preferably carried out at 300°C and 600 °C for 1h respectively.

Wherein, the temperature of the sintering is preferably 1030-1080°C, for example 1040°C.

Wherein, the time of the sintering is conventional in the field, for example 2h.

Wherein, before the cooling, Ar gas can be introduced to make the pressure reach 0.1 Mpa.

In the present disclosure, after the sintering and before the ageing treatment, a grain boundary diffusion treatment is further carried out preferably.

Wherein, the operations and conditions of the grain boundary diffusion can be conventional in the field. For example, the surface of the neodymium-iron-boron magnet material are attached with Tb-containing substance and/or Dy-containing substance by evaporating, coating or sputtering, and subjected to diffusion heat treatment.

The Tb-containing substance can be a Tb metal, a Tb-containing compound, for example a Tb-containing fluoride or alloy.

The Dy-containing substance can be a Dy metal, a Dy-containing compound, for example a Dy-containing fluoride or alloy.

The temperature of the diffusion heat treatment may be 800-900°C, for example 850°C.

The time of the diffusion heat treatment can be 12-48h, for example 24h.

In the present disclosure, in the ageing treatment, the temperature of secondary ageing treatment is preferably 520-650°C, for example 550°C.

In the present disclosure, in the secondary ageing treatment, heating rate to 550-650°C is preferably 3-5°C/min. The starting point of heating can be room temperature.

In the present disclosure, the room temperature is 25°C±5°C.

The present disclosure further provides a neodymium-iron-boron magnet material, which is prepared by the preparation method mentioned above.

The present disclosure provides a neodymium-iron-boron magnet material, the neodymium-iron-boron magnet material comprises the following components by mass percentage:
29.4-32.6% of R', R' includes Pr and Nd; wherein, Pr ≥17.14%;
Cu >_ 0.34%;
0.9-1.2% of B;
64-69.2% of Fe;
the percentage refers to the mass percentage relative to the total mass of the neodymium-iron-boron magnet material.

In the present disclosure, the content of Pr is preferably 17.14-26.1%, for example 17.149%, 17.15%, 17.154%, 18.15%, 18.152%, 18.154%, 18.155%, 19.15%, 19.152%, 19.154%, 19.155%, 19.159%, 20.13%, 20.155%, 20.16%, 21.157%, 22.15%, 22.151%, 22.152%, 22.1555%, 23.15%, 24.151%, 24.152%, 24.155%, 24.157%, 24.158%, 25.15%, 25.152%, 25.153%, 25.156% or 26.01%, the percentage refers to the mass percentage relative to the total mass of the neodymium-iron-boron magnet material.

In the present disclosure, the content of Nd is preferably 15% or less, more preferably 4-13%, for example 4.02%, 5.847%, 5.84%, 5.849%, 5.85%, 5.851%, 5.852%, 5.853%, 5.854%, 6.851%, 6.852%, 6.853%, 7.85%, 8.846%, 8.847%, 8.85%, 8.851%, 8.852%, 8.853%, 9.85%, 9.851%, 10.844%, 10.846%, 10.849%, 11.349%, 11.384%, 12.341%, 12.345%, 12.348%, 12.35%, 12.351% ,12.364%, 12.791%, 12.802% or 12.849%, the percentage refers to the mass percentage relative to the total mass of the neodymium-iron-boron magnet material.

In the present disclosure, the ratio of the mass of Nd to the total mass of R' is preferably less than 0.5, more preferably 0.1-0.45, for example 0.1, 0.12, 0.13, 0.18, 0.2, 0.21, 0.23, 0.24, 0.25, 0.26, 0.27, 0.3, 0.31, 0.37, 0.38, 0.4, 0.41 or 0.42.

In the present disclosure, the content of R' is preferably 29.49-32.53%, for example 29.495%, 29.501%, 30.003%, 30.004%, 30.03%, 30.441%, 30.517%, 30.518%, 30.957%, 30.98%, 31%, 31.006%, 31.0065%, 31.009%, 31.011%, 31.012%, 31.013%, 31.498%, 31.504%, 31.539%, 31.946%, 31.972%, 31.977%, 31.995%, 31.999%, 32%, 32.001%, 32.013%, 32.015%, 32.021%, 32.022%, 32.023%, 32.024%, 32.025%, 32.026%, 32.027%, 32.04%, 32.043%, 32.437% or 32.521%, the percentage refers to the mass percentage relative to the total mass of the neodymium-iron-boron magnet material.

In the present disclosure, preferably, R' further comprises other rare earth elements besides Pr and Nd, for example Y.

In the present disclosure, preferably, R' further comprises RH, RH is a heavy rare earth element, the kind of RH preferably comprises one or more of Dy, Tb and Ho, more preferably Dy and/or Tb.

Wherein, the mass ratio of RH and R' is preferably less than 0.253, preferably 0-0.07, for example 1.01/32.015, 1.02/30.517, 1.02/32.021, 1.02/32.023, 1.02/32.024, 1.02/32.024, 1.02/32.025, 1.02/32.025, 1.02/32.026, 1.03/32.04, 1.04/32.043, 1.432/32.437, 1.46/30.441, 1.47/31.972, 1.48/31.977, 1.5/32, 1.52/32.521, 1.98/30.98, 1.99/31.995, 1/31.999, 1/32,2.01/31.011, 2.01/31.013, 2.01/32.013, 2.02/32.022, 2.02/32.027, 2/31 or 2/31.012.

Wherein, the content of RH is preferably 1-2.5%, for example 1%, 1.01%, 1.02%, 1.03%, 1.04%, 1.432%, 1.46%, 1.47%, 1.48%, 1.5%, 1.52%, 1.98%, 1.99%, 2%, 2.01% or 2.02%, the percentage refers to the mass percentage relative to the total mass of the neodymium-iron-boron magnet material.

When RH comprises Tb, the content of Tb is preferably 0.5-2wt.%, for example 0.7%, 0.72%, 0.82%, 0.9%, 0.91%, 1%, 1.02%, 1.47%, 1.48%, 1.5%, 1.81%, 1.88%, 1.89%, 1.9%, 1.91% or 2.01%, the percentage refers to the mass percentage relative to the total mass of the neodymium-iron-boron magnet material.

When RH comprises Dy, the content of Dy is preferably 0.5wt.% or less, for example 0.1%, 0.2%, 0.21%, 0.3%, 0.31% or 0.312%, the percentage refers to the mass percentage relative to the total mass of the neodymium-iron-boron magnet material.

When RH comprises Ho, the content of Ho is a conventional content in the field, usually 0.8-2%, for example 0.98%, 0.99% or 1%, the percentage refers to the mass percentage relative to the total mass of the neodymium-iron-boron magnet material.

In the present disclosure, the content of Cu is preferably 0.34-1.3%, for example 0.341%, 0.41%, 0.452%, 0.47%, 0.502%, 0.51%, 0.52%, 0.598%, 0.62%, 0.648%, 0.649%, 0.701%, 0.702%, 0.71%, 0.78%, 0.79%, 0.795%, 0.806%, 0.81%, 0.852%, 0.89%, 0.901%, 0.903%, 0.91%, 0.92%, 0.948%, 1.021%, 1.05%, 1.08%, 1.101%, 1.103%, 1.12%, 1.18%, 1.19%, 1.202% or 1.21%, the percentage refers to the mass percentage relative to the total mass of the neodymium-iron-boron magnet material.

In the present disclosure, the content of B is preferably 0.95-1.2%, for example 0.983%, 0.984%, 0.985%, 0.988%, 0.989%, 1.02% or 1.19%, the percentage refers to the mass percentage relative to the total mass of the neodymium-iron-boron magnet material.

In the present disclosure, the content of Fe is preferably 64.8-69.2%, for example 64.965% ,65.031%, 65.095%, 65.155%, 65.204%, 65.36%, 65.4%, 65.458%, 65.525%, 65.626%, 65.63%, 65.686%, 65.817%, 65.8395%, 65.869%, 65.909%, 65.963%, 65.994%, 65.995%, 66.039%, 66.04%, 66.099%, 66.157%, 66.218%, 66.267%, 66.364%, 66.377%, 66.427%, 66.437%, 66.52%, 66.605%, 66.671%, 66.8075%, 66.81%, 66.87%, 67.095%, 67.12%, 67.137%, 67.457%, 67.578%, 67.996%, 68.302%, 68.556% or 69.181%, the percentage refers to the mass percentage relative to the total mass of the neodymium-iron-boron magnet material.

In the present disclosure, preferably, the neodymium-iron-boron magnet material further comprises Al.

In the present disclosure, the content of Al is preferably 0.5% or less, more preferably 0.03-0.5wt.%, for example 0.01%, 0.02%, 0.03%, 0.1%, 0.102%, 0.12%, 0.2%, 0.21%, 0.24%, 0.25%, 0.29%, 0.3%, 0.31%, 0.38%, 0.4%, 0.42%, 0.45%, 0.46% or 0.48%, the percentage refers to the mass percentage relative to the total mass of the neodymium-iron-boron magnet material.

In the present disclosure, preferably, the neodymium-iron-boron magnet material further comprises Zr.

In the present disclosure, the content of Zr is preferably 0.05-0.31wt.%, for example 0.1%, 0.21%, 0.22%, 0.25%, 0.251%, 0.252%, 0.261%, 0.272%, 0.28%, 0.281%, 0.282%, 0.291% 0.3% or 0.301%, more preferably 0.25-0.31, the percentage refers to the mass percentage of each component relative to the total mass of the neodymium-iron-boron magnet material.

In the present disclosure, preferably, the neodymium-iron-boron magnet material further comprises Ga.

Wherein, the content of Ga is preferably 0.51% or less, more preferably 0.1-0.51%, for example 0.1%, 0.101%, 0.102%, 0.11%, 0.12%, 0.152%, 0.18%, 0.2%, 0.202%, 0.24%, 0.25%, 0.251%, 0.302%, 0.401% or 0.501%, the percentage refers to the mass percentage of each component relative to the total mass of the neodymium-iron-boron magnet material.

In the present disclosure, preferably, the neodymium-iron-boron magnet material further comprises Co.

Wherein, the content of Co is preferably 0.2-1.5%, for example 0.2% or 1%, the percentage refers to the mass percentage of each component relative to the total mass of the neodymium-iron-boron magnet material.

In the present disclosure, preferably, the neodymium-iron-boron magnet material further comprises O.

Wherein, the content of O is preferably 0.13% or less, the percentage refers to the mass percentage of each component relative to the total mass of the neodymium-iron-boron magnet material.

In the present disclosure, the neodymium-iron-boron magnet material can further comprise other conventional elements in the field, for example one or more of Zn, Ag, In, Sn, V, Cr, Nb, Ti, Mo, Ta, Hf and W.

Wherein, the content of Zn can be a conventional content in the field, preferably 0.02-0.08%, for example 0.03%, 0.04% or 0.07%, the percentage refers to the mass percentage of each component relative to the total mass of the neodymium-iron-boron magnet material.

Wherein, the content of Mo can be a conventional content in the field, preferably 0.01-0.08%, for example 0.03%, 0.06% or 0.07%, the percentage refers to the mass percentage of each component relative to the total mass of the neodymium-iron-boron magnet material.

In the present disclosure, the neodymium-iron-boron magnet material preferably comprises the following components by mass percentage: 29.4-32.6% of R', R' is a rare earth element and includes Pr and Nd; wherein, Pr ≥17.14%; Cu ≥0.34%; Al≤0.5%; 0.9-1.2% of B; 64-69.2% of Fe; more preferably, the content of Pr is 17.14-26.1%; more preferably, the content of Cu is preferably 0.35-1.2%; more preferably, R' further comprises RH, RH is a heavy rare earth element, the content of the heavy rare earth element is preferably 1-2.5%, the percentage refers to the mass percentage relative to the total mass of the neodymium-iron-boron magnet material.

In the present disclosure, the neodymium-iron-boron magnet material preferably comprises the following components by mass percentage: 29.4-32.6% of R', R' is a rare earth element and includes Pr and Nd; wherein, Pr ≥17.15%; Cu ≥0.34%; 0.25-0.3% of Zr; 0.9-1.2% of B; 64-69.2% of Fe; more preferably, the content of Pr is 17.14-26.1%; more preferably, the content of Cu is preferably 0.35-1.2%; more preferably, R' further comprises RH, RH is a heavy rare earth element, the content of the heavy rare earth element is preferably 1-2.5%, the percentage refers to the mass percentage relative to the total mass of the neodymium-iron-boron magnet material.

In the present disclosure, the neodymium-iron-boron magnet material preferably comprises the following components by mass percentage: 29.4-32.6% of R', R' is a rare earth element and includes Pr and Nd; wherein, Pr ≥17.14%; Cu ≥0.34%; Al<0.5%; 0.25-0.3% of Zr; 0.9-1.2% of B; 64-69.2% of Fe; more preferably, the content of Pr is 17.14-26.1%; more preferably, the content of Cu is preferably 0.35-1.2%; more preferably, R' further comprises RH, RH is a heavy rare earth element, the content of the heavy rare earth element is preferably 1-2.5%; the kind of RH preferably comprises Dy and/or Tb, wherein, the content of Tb is preferably 0.5-2%, the content of Dy is preferably 1% or less; the percentage refers to the mass percentage relative to the total mass of the neodymium-iron-boron magnet material.

In the present disclosure, the neodymium-iron-boron magnet material preferably comprises the following components by mass percentage: 29.4-32.6% of R', R' is a rare earth element and includes Pr and Nd; wherein, Pr ≥17.14%; Cu ≥0.34%; Ga≤0.42%; 0.9-1.2% of B; 64-69.2% of Fe; more preferably, the content of Pr is 17.14-26.1%; more preferably, the content of Cu is preferably 0.35-1.3%; more preferably, R' further comprises RH, RH is a heavy rare earth element, the content of the heavy rare earth element is preferably 1-2.5%, the percentage refers to the mass percentage relative to the total mass of the neodymium-iron-boron magnet material.

In the present disclosure, the neodymium-iron-boron magnet material preferably comprises the following components by mass percentage: 29.4-32.6% of R', R' is a rare earth element and includes Pr and Nd; wherein, Pr ≥17.14%; Cu ≥0.34%; Al<0.5%; Ga≤0.42%; 0.9-1.2% of B; 64-69.2% of Fe; more preferably, the content of Pr is 17.14-26.1%; more preferably, the content of Cu is preferably 0.35-1.3%; more preferably, R' further comprises RH, RH is a heavy rare earth element, the content of the heavy rare earth element is preferably 1-2.5%, the percentage refers to the mass percentage relative to the total mass of the neodymium-iron-boron magnet material.

In the present disclosure, the neodymium-iron-boron magnet material comprises the following components by mass percentage: 29.4-32.6% of R', R' is a rare earth element and includes Pr and Nd; wherein, Pr ≥17.14%; Cu ≥0.34%; Ga≤0.42%;0.25-0.3% of Zr; 0.9-1.2% of B; 64-69.2% of Fe; more preferably, the content of Pr is 17.14-26.1%; more preferably, the content of Cu is preferably 0.35-1.3%, more preferably, R' further comprises RH, RH is a heavy rare earth element, the content of the heavy rare earth element is preferably 1-2.5%, the percentage refers to the mass percentage relative to the total mass of the neodymium-iron-boron magnet material.

In the present disclosure, the raw material composition of neodymium-iron-boron magnet material comprises the following components by mass percentage: 29.4-32.6% of R', R' is a rare earth element and includes Pr and Nd; wherein, Pr ≥17.14%; Cu ≥0.34%; Al≤0.5%; Ga≤0.42%; 0.25-0.3% of Zr; 0.9-1.2% of B; 64-69.2% of Fe; more preferably, the content of Pr is 17.14-26.1%; more preferably, the content of Cu is preferably 0.35-1.3%, more preferably, R' further comprises RH, RH is a heavy rare earth element, the content of the heavy rare earth element is preferably 1-2.5%; the kind of RH preferably comprises Dy and/or Tb, wherein, the content of Tb is preferably 0.5-2%, the content of Dy is preferably 1% or less; the percentage refers to the mass percentage relative to the total mass of the neodymium-iron-boron magnet material.

In the present disclosure, the percentage refers to the mass percentage of each component relative to the total mass of the neodymium-iron-boron magnet material.

The present disclosure further provides a neodymium-iron-boron magnet material, in the intergranular triangle region of the neodymium-iron-boron magnet material, the ratio of the total mass of Pr and Cu to the total mass of each element in the intergranular triangle region is Q1; at the grain boundary of the neodymium-iron-boron magnet material, the ratio of the total mass of Pr and Cu to the total mass of each element at the grain boundary is Q2; wherein, Q1 < Q2, and Q2 ≥ 0.1; and
wherein the components of the neodymium-iron-boron magnet material refer to those of the neodymium-iron-boron magnet material mentioned above.

In the present disclosure, the grain boundary refers to the boundary between two grains, and the intergranular triangle is the gap formed by three and more grains.

The present disclosure further provides a use of the neodymium-iron-boron magnet material as an electronic component in a motor.

In the present disclosure, the motor is preferably a new energy vehicle drive motor, an air-conditioning compressor or an industrial servo motor, a wind turbine, an energy-saving elevator or a loudspeaker assembly.

Based on the common sense in the field, the preferred conditions of the preparation methods can be combined arbitrarily to obtain preferred examples of the present disclosure.

The reagents and raw materials used in the invention are commercially available.

The positive progress of the present invention is that the neodymium-iron-boron magnet material of the present invention simultaneously increases the content of praseodymium and copper, so that the grain boundary phase is clearer, and the obtained neodymium-iron-boron magnet material has higher remanence and coercive force.

### Brief description of the drawings

Fig.1 is the distribution diagram of Pr, Nd, Cu, Ti, Co and O elements formed by the FE-EPMA face scan of the neodymium-iron-boron magnet material prepared in Example 10.
Fig. 2 is the distribution diagram of elements at the grain boundary of the neodymium-iron-boron magnet material in Example 10, and symbol 1 in Fig. 2 is the point taken in quantitative analysis at the grain boundary.
Fig. 3 is the distribution diagram of elements in the intergranular triangle of the neodymium-iron-boron magnet material in Example 10, and symbol 1 in Fig. 3 is the point taken in quantitative analysis at the grain boundary.

### Detailed description of the preferred embodiment

The following examples further illustrate the present disclosure, but the present disclosure is not limited thereto. Experiment methods in which specific conditions are not indicated in the following embodiments are selected according to conventional methods and conditions, or according to the product specification. In the table below, wt.% refers to the mass percentage of the component in the raw material composition of the R-T-B permanent magnet material, and "/" indicates that the element has not been added. "Br" is the residual magnetic flux density and "Hcj" is the intrinsic coercivity.

The formulations for the raw material compositions of the neodymium-iron-boron magnet material in each Example and Comparative Example are shown in Table 1 below.

**Table 1 The formulations for the raw material compositions of the neodymium-iron-boron magnet material in each Example and Comparative Example (wt.%)**

| No. | Nd | Pr | Dy | Tb | Ho | Cu | Al | Ga | Zr | Co | Zn | Mo | B | Fe |
|---|---|---|---|---|---|---|---|---|---|---|---|---|---|---|
| 1 | 12.35 | 17.15 | / | / | / | 0.35 | / | / | / | / | / | / | 0.985 | 69.165 |
| 2 | 12.85 | 17.15 | / | / | / | 0.45 | / | / | / | / | / | / | 0.985 | 68.565 |
| 3 | 12.35 | 18.15 | / | / | / | 0.5 | / | / | / | / | / | / | 0.985 | 68.015 |
| 4 | 12.85 | 18.15 | / | / | / | 0.6 | / | / | / | / | / | / | 0.985 | 67.415 |
| 5 | 12.35 | 19.15 | / | / | / | 0.65 | / | / | / | / | / | / | 0.985 | 66.865 |
| 6 | 12.85 | 19.15 | / | / | / | 0.7 | / | / | / | / | / | / | 0.985 | 66.315 |
| 7 | 11.35 | 20.15 | / | / | / | 0.8 | / | / | / | / | / | / | 0.985 | 66.715 |
| 8 | 11.35 | 20.15 | / | / | / | 0.9 | / | / | / | / | / | / | 0.985 | 66.615 |
| 9 | 10.85 | 21.15 | / | / | / | 1 | / | / | / | / | / | / | 0.985 | 66.015 |
| 10 | 4 | 26 | / | / | / | 1.1 | / | / | 0.1 | 0.2 | / | / | 0.985 | 67.615 |
| 11 | 8.85 | 22.15 | / | / | / | 1.2 | / | / | / | / | / | / | 0.985 | 66.815 |
| 12 | 5.85 | 25.15 | 0.3 | 0.7 | / | 0.5 | 0.03 | / | / | / | / | / | 0.985 | 66.485 |
| 13 | 5.85 | 25.15 | / | 1 | / | 0.7 | 0.1 | / | / | / | / | / | 0.985 | 66.215 |
| 14 | 5.85 | 24.15 | 0.2 | 1.8 | / | 0.9 | 0.2 | / | / | / | / | / | 0.985 | 65.915 |
| 15 | 5.85 | 24.15 | / | 2 | / | 1.1 | 0.25 | / | / | / | / | / | 0.985 | 65.665 |
| 16 | 8.85 | 22.15 | 0.2 | 0.8 | / | 1.2 | / | 0.1 | / | / | / | / | 0.985 | 65.715 |
| 17 | 8.85 | 22.15 | 0 | 1 | / | 0.85 | / | 0.2 | / | / | / | / | 0.985 | 65.965 |
| 18 | 7.85 | 23.15 | 0.1 | 0.9 | / | 0.65 | / | / | 0.1 | / | / | / | 0.985 | 66.265 |
| 19 | 7.85 | 23.15 | 0.1 | 0.9 | / | 0.95 | / | / | 0.25 | / | / | / | 0.985 | 65.815 |
| 20 | 12.35 | 18.15 | / | 1.5 | / | 1.05 | / | / | / | 1 | | | 0.985 | 64.965 |
| 21 | 10.85 | 19.15 | 0.1 | 1.9 | / | 0.8 | 0.1 | 0.1 | / | / | / | / | 0.985 | 66.015 |
| 22 | 10.85 | 19.15 | 0.1 | 1.9 | / | 0.9 | 0.3 | 0.2 | / | / | / | / | 0.985 | 65.615 |
| 23 | 12.35 | 18.15 | / | 1.5 | / | 0.5 | / | 0.25 | 0.22 | / | / | / | 0.985 | 66.045 |
| 24 | 12.35 | 18.15 | / | 1.5 | / | 0.6 | / | 0.1 | 0.28 | / | / | / | 0.985 | 66.035 |
| 25 | 9.85 | 19.15 | 0.1 | 1.9 | / | 1.2 | 0.2 | / | 0.25 | / | / | / | 0.985 | 66.365 |
| 26 | 9.85 | 19.15 | 0.1 | 1.9 | / | 0.8 | 0.4 | / | 0.3 | / | / | / | 0.985 | 66.515 |
| 27 | 8.85 | 22.15 | 0.1 | 0.9 | / | 0.9 | 0.3 | / | 0.26 | / | / | / | 1 | 65.54 |
| 28 | 5.85 | 25.15 | 0.2 | 0.8 | / | 1.2 | 0.46 | / | 0.29 | / | | | 0.985 | 65.065 |
| 29 | 5.85 | 25.15 | 0.3 | 0.7 | / | 1.1 | 0.48 | / | 0.3 | / | | | 0.985 | 65.135 |
| 30 | 9.85 | 19.15 | 0.1 | 1.9 | / | 0.6 | 0.2 | 0.15 | 0.2 | / | | | 0.985 | 66.865 |
| 31 | 8.85 | 22.15 | 0.3 | 0.7 | / | 0.8 | 0.3 | 0.18 | 0.25 | / | | | 0.985 | 65.485 |
| 32 | 6.85 | 24.15 | / | / | / | 0.8 | 0.4 | 0.2 | 0.27 | / | | | 1.1 | 66.23 |
| 33 | 6.85 | 24.15 | / | / | / | 0.9 | 0.45 | 0.2 | 0.28 | / | | | 1.2 | 65.93 |
| 34 | 9.85 | 19.15 | / | 2 | / | 0.4 | 0.1 | 0.1 | 0.25 | | | | 0.985 | 67.165 |
| 35 | 6.85 | 24.15 | / | 1 | / | 0.5 | 0.25 | 0.1 | 0.3 | | | | 0.985 | 65.865 |
| 36 | 12.35 | 17.15 | | | | 0.7 | 0.02 | 0.25 | 0.25 | | | | 0.985 | 68.295 |
| 37 | 12.35 | 17.15 | | 1 | | 0.8 | 0.02 | 0.3 | 0.25 | | | | 0.985 | 67.145 |
| 38 | 8.85 | 22.15 | 0.3 | 0.7 | | 0.9 | 0.03 | 0.4 | 0.28 | | | | 0.985 | 65.405 |
| 39 | 8.85 | 22.15 | 0.3 | 0.7 | | 1.1 | 0.03 | 0.5 | 0.3 | | | | 0.985 | 65.085 |
| 40 | 8.85 | 20.15 | 0.3 | 0.7 | 1.0 | 0.8 | 0.3 | 0 | 0.25 | / | 0.04 | 0.08 | 0.985 | 66.545 |
| 41 | 8.85 | 20.15 | 0.3 | 0.7 | 1.0 | 0.9 | 0.3 | 0 | 0.25 | / | 0.08 | 0.04 | 0.985 | 66.445 |
| 42 | 6.85 | 24.15 | / | / | 1.0 | 0.9 | 0.4 | 0 | 0.25 | / | 0.05 | 0.05 | 0.985 | 65.365 |
| 45 | 5.85 | 25.15 | / | 1 | / | 0.2 | 0.1 | / | / | / | / | / | 0.985 | 66.715 |
| 46 | 5.85 | 25.15 | / | 1 | / | 0.1 | 0.1 | / | / | / | / | / | 0.985 | 66.815 |
| 47 | 14.85 | 15.15 | | | / | 0.9 | 0.2 | / | / | / | / | / | 0.985 | 67.915 |
| 48 | 21.15 | 8.85 | | | / | 0.9 | 0.2 | / | / | / | / | / | 0.985 | 67.915 |

### Example 1

The neodymium-iron-boron magnet material is prepared as follows:
(1) Melting and casting process: according to the formulation shown in Table 1, the prepared raw material was put into a crucible made of alumina and vacuum melted in a high frequency vacuum induction melting furnace and in a vacuum of 5×10⁻² Pa at a temperature of 1500°C or less. After the vacuum melting, Ar gas was introduced into the melting furnace to make the pressure of furnace reach 55,000 Pa, casting was carried out, and the quenched alloy was obtained at a cooling rate of 10²°C/sec to 10⁴°C/sec.
(2) Hydrogen decrepitation process: the melting furnace in which the quench alloy was placed was evacuated at room temperature, and then hydrogen of 99.9% purity was introduced into the furnace for hydrogen decrepitation to maintain the hydrogen pressure at 0.15Mpa; after full hydrogen absorption, vacuuming was conducted while heating up to fully dehydrogenate; then cooling was carried out and the powder after hydrogen decrepitation was taken out.
(3) Micro pulverization process: the powder after hydrogen decrepitation was pulverized by jet mill for 3 hours under a nitrogen atmosphere with an oxidizing gas content of 150ppm or less and under a pressure of 0.38MPa in the pulverization chamber to obtain a fine powder. The oxidizing gas referred to oxygen or moisture.
(4) Zinc stearate was added to the powder from jet mill pulverization, and the addition amount of zinc stearate was 0.12% of the weight of the mixed powder, and then mixed thoroughly with a V-mixer.
(5) Magnetic field forming process: the above-mentioned zinc stearate added powder was formed into a first cube with a side length of 25 mm by using a right-angle oriented magnetic field forming machine at an oriented magnetic field of 1.6 T and a forming pressure of 0.35 ton/cm²; and it was demagnetised in a magnetic field of 0.2 T after the first forming. In order to prevent the formed body obtained after the first forming from being exposed to air, it was sealed, and then a secondary forming machine (isostatic forming machine) was used to perform secondary forming at a pressure of 1.3 ton/cm².
(6) Sintering process: each formed body was moved to the sintering furnace for sintering, which was held in vacuum of 5×10⁻³ Pa at 300°C and 600°C for 1 hour respectively; then, sintered at 1040°C for 2 hours; then cooled to room temperature after the pressure reached 0.1 Mpa by introducing Ar gas.
(7) Ageing treatment process: the sintered body was heat treated in high purity Ar gas at 550°C for 3 hours and then it was cooled to room temperature before being taken out.

The preparation process of Example 2-42 and Comparative Examples 45-48 was the same as that of Example 1.

Example 43 and 44 employed Tb grain boundary diffusion method in the preparation process.

The raw material compositions of No. 12 and 16 in Table 1 were first prepared according to the preparation of the sintered body of Example 1 to obtain a sintered body, followed by grain boundary diffusion, and then ageing treatment was carried out. The ageing treatment process was the same as in Example 1, and the process of grain boundary diffusion was as follows.

The sintered body was processed into a magnet with a diameter of 20 mm and a sheet thickness of less than 7 mm in the direction of the magnetic field orientation, and after surface cleaning, the magnet was coated with a full spray using a raw material prepared with Tb fluoride, respectively, and the coated magnet was dried and the metal with Tb element attached was sputtered on the magnet surface in a high purity Ar atmosphere at the temperature of 850°C diffusion heat treatment for 24 hours. Cool to room temperature.

### Examples of effect implementation

The magnetic properties and compositions of the neodymium-iron-boron magnet materials produced in each example and comparative example were measured and the crystalline phase structure of the magnets is observed by FE-EPMA.
(1) Magnetic properties evaluation: The magnet materials were tested for magnetic properties by using the NIM-10000H BH bulk rare earth permanent magnet non-destructive measurement system from the China Metrology Institute. The results of the magnetic properties testing were shown in Table 2 below.

**Table 2**

| No. | Br(kGs) | Hcj(kOe) | 80°C Hcj Absolute value of temperature coefficient | 150°C Hcj Absolute value of temperature coefficient | 180°C Hcj Absolute value of temperature coefficient |
|---|---|---|---|---|---|
| 1 | 14.35 | 17.01 | 0.689 | / | / |
| 2 | 14.16 | 17.62 | 0.684 | / | / |
| 3 | 13.98 | 18.03 | 0.679 | / | / |
| 4 | 14.01 | 18.21 | 0.674 | / | / |
| 5 | 13.84 | 18.56 | 0.672 | / | / |
| 6 | 13.65 | 18.88 | 0.668 | / | / |
| 7 | 13.7 | 19.15 | 0.663 | / | / |
| 8 | 13.62 | 19.39 | 0.663 | / | / |
| 9 | 13.5 | 20.11 | 0.652 | / | / |
| 10 | 13.49 | 20.64 | 0.648 | / | / |
| 11 | 13.7 | 22 | 0.621 | / | / |
| 12 | 13.30 | 23.6 | 0.601 | / | / |
| 13 | 13.19 | 25.24 | / | 0.515 | / |
| 14 | 13.06 | 28.02 | / | 0.485 | / |
| 15 | 13.00 | 28.98 | / | 0.479 | / |
| 16 | 13.59 | 24.48 | / | 0.523 | / |
| 17 | 13.25 | 24.68 | / | 0.520 | / |
| 18 | 13.29 | 22.73 | 0.619 | / | / |
| 19 | 13.15 | 24.03 | / | 0.520 | / |
| 20 | 13.02 | 25.23 | | 0.515 | |
| 21 | 13.27 | 26.81 | / | 0.512 | / |
| 22 | 13.07 | 28.71 | / | 0.491 | / |
| 23 | 13.34 | 25.66 | / | 0.519 | / |
| 24 | 13.29 | 25.08 | / | 0.522 | / |
| 25 | 13.39 | 27.24 | | 0.493 | / |
| 26 | 12.91 | 27.09 | | 0.503 | |
| 27 | 13.29 | 24.69 | / | 0.531 | / |
| 28 | 13.01 | 26.97 | / | 0.508 | / |
| 29 | 12.66 | 26.84 | | 0.511 | |
| 30 | 13.15 | 26.87 | / | 0.504 | / |
| 31 | 13.14 | 26.05 | / | 0.510 | / |
| 32 | 13.10 | 26.68 | / | 0.509 | / |
| 33 | 13.59 | 23.93 | 0.591 | / | / |
| 34 | 13.42 | 24.47 | / | 0.524 | / |
| 35 | 13.18 | 23.73 | 0.593 | / | / |
| 36 | 14.33 | 18.76 | 0.675 | / | / |
| 37 | 13.74 | 23.39 | 0.599 | / | / |
| 38 | 13.19 | 26.04 | / | 0.510 | / |
| 39 | 12.95 | 27.52 | / | 0.488 | / |
| 40 | 12.75 | 24.19 | / | 0.521 | / |
| 41 | 12.79 | 24.23 | / | 0.519 | / |
| 42 | 12.63 | 23.72 | 0.594 | / | / |
| 43 | 13.02 | 33.2 | / | / | 0.428 |
| 44 | 13.37 | 34.8 | / | / | 0 |
| 45 | 13.27 | 21.75 | 0.629 | / | / |
| 46 | 13.30 | 21.53 | 0.632 | / | / |
| 47 | 13.8 | 16.8 | 0.742 | / | / |
| 48 | 14.0 | 14.9 | 0.782 | / | / |

(2) Component determination: each component was determined by using a high frequency inductively coupled plasma emission spectrometer (ICP-OES). The component determination results were shown in Table 3 below.

**Table 3**

| No. | Nd | Pr | Dy | Tb | Ho | Cu | Al | Ga | Zr | Co | Zn | Mo | B | Fe |
|---|---|---|---|---|---|---|---|---|---|---|---|---|---|---|
| 1 | 12.341 | 17.154 | / | / | / | 0.341 | / | / | / | / | / | / | 0.983 | 69.181 |
| 2 | 12.849 | 17.154 | / | / | / | 0.452 | / | / | / | / | / | / | 0.989 | 68.556 |
| 3 | 12.364 | 18.154 | / | / | / | 0.502 | / | / | / | / | / | / | 0.984 | 67.996 |
| 4 | 12.802 | 18.155 | / | / | / | 0.598 | / | / | / | / | / | / | 0.988 | 67.457 |
| 5 | 12.348 | 19.15 | / | / | / | 0.649 | / | / | / | / | / | / | 0.983 | 66.87 |
| 6 | 12.791 | 19.155 | / | / | / | 0.701 | / | / | / | / | / | / | 0.989 | 66.364 |
| 7 | 11.384 | 20.155 | / | / | / | 0.806 | / | / | / | / | / | / | 0.984 | 66.671 |
| 8 | 11.349 | 20.155 | / | / | / | 0.903 | / | / | / | / | / | / | 0.988 | 66.605 |
| 9 | 10.844 | 21.157 | / | / | / | 1.021 | / | / | / | / | / | / | 0.983 | 65.995 |
| 10 | 4.02 | 26.01 | / | / | / | 1.103 | / | / | 0.1 | 0.2 | / | / | 0.989 | 67.578 |
| 11 | 8.851 | 22.1555 | / | / | / | 1.202 | / | / | / | / | / | / | 0.984 | 66.8075 |
| 12 | 5.854 | 25.156 | 0.31 | 0.72 | / | 0.52 | 0.02 | / | / | / | / | / | 0.983 | 66.437 |
| 13 | 5.848 | 25.156 | / | 1.02 | / | 0.71 | 0.12 | / | / | / | / | / | 0.989 | 66.157 |
| 14 | 5.849 | 24.158 | 0.21 | 1.81 | / | 0.91 | 0.21 | / | / | / | / | / | 0.984 | 65.869 |
| 15 | 5.847 | 24.155 | / | 2.02 | / | 1.12 | 0.24 | / | / | / | / | / | 0.988 | 65.63 |
| 16 | 8.846 | 22.155 | 0.2 | 0.82 | / | 1.19 | / | 0.12 | / | / | / | / | 0.983 | 65.686 |
| 17 | 8.85 | 22.15 | 0 | 1 | / | 0.852 | / | 0.2 | / | / | / | / | 0.985 | 65.963 |
| 18 | 7.85 | 23.15 | 0.1 | 0.9 | / | 0.648 | / | / | 0.1 | / | / | / | 0.985 | 66.267 |
| 19 | 7.85 | 23.15 | 0.1 | 0.9 | / | 0.948 | / | / | 0.25 | / | / | / | 0.985 | 65.817 |
| 20 | 12.35 | 18.15 | / | 1.5 | / | 1.05 | / | / | / | 1 | | | 0.985 | 64.965 |
| 21 | 10.849 | 19.154 | 0.1 | 1.91 | / | 0.81 | 0.1 | 0.1 | / | / | / | / | 0.983 | 65.994 |
| 22 | 10.846 | 19.159 | 0.1 | 1.89 | / | 0.89 | 0.3 | 0.2 | / | / | / | / | 0.989 | 65.626 |
| 23 | 12.345 | 18.152 | / | 1.48 | / | 0.47 | / | 0.25 | 0.22 | / | / | / | 0.984 | 66.099 |
| 24 | 12.35 | 18.152 | / | 1.47 | / | 0.62 | / | 0.1 | 0.28 | / | / | / | 0.988 | 66.04 |
| 25 | 9.85 | 19.15 | 0.1 | 1.88 | / | 1.21 | 0.2 | / | 0.25 | / | / | / | 0.983 | 66.377 |
| 26 | 9.85 | 19.15 | 0.1 | 1.9 | / | 0.795 | 0.4 | / | 0.3 | / | / | / | 0.985 | 66.52 |
| 27 | 8.853 | 22.152 | 0.1 | 0.91 | / | 0.91 | 0.3 | / | 0.261 | / | / | / | 0.989 | 65.525 |
| 28 | 5.851 | 25.153 | 0.2 | 0.82 | / | 1.21 | 0.46 | / | 0.291 | / | / | / | 0.984 | 65.031 |
| 29 | 5.85 | 25.15 | 0.3 | 0.7 | / | 1.08 | 0.48 | / | 0.3 | / | / | / | 0.985 | 65.155 |
| 30 | 9.851 | 19.152 | 0.1 | 1.91 | / | 0.62 | 0.21 | 0.152 | 0.21 | / | / | / | 0.985 | 66.81 |
| 31 | 8.853 | 22.152 | 0.3 | 0.72 | / | 0.81 | 0.29 | 0.18 | 0.252 | / | / | / | 0.985 | 65.458 |
| 32 | 6.851 | 24.155 | / | / | / | 0.78 | 0.42 | 0.202 | 0.272 | / | / | / | 1.102 | 66.218 |
| 33 | 6.852 | 24.157 | / | / | / | 0.92 | 0.45 | 0.24 | 0.282 | / | / | / | 1.19 | 65.909 |
| 34 | 9.851 | 19.15 | / | 2.01 | / | 0.41 | 0.102 | 0.101 | 0.251 | / | / | / | 0.988 | 67.137 |
| 35 | 6.852 | 24.151 | / | 1.02 | / | 0.502 | 0.250 | 0.102 | 0.301 | / | / | / | 0.983 | 65.839 |
| 36 | 12.351 | 17.150 | / | / | / | 0.702 | 0.01 | 0.251 | 0.251 | / | / | / | 0.983 | 68.302 |
| 37 | 12.348 | 17.149 | / | 1.02 | / | 0.79 | 0.03 | 0.302 | 0.252 | / | / | / | 0.989 | 67.12 |
| 38 | 8.848 | 22.151 | 0.3 | 0.7 | / | 0.901 | 0.03 | 0.401 | 0.281 | / | / | / | 0.988 | 65.4 |
| 39 | 8.847 | 22.152 | 0.3 | 0.7 | / | 1.101 | 0.02 | 0.501 | 0.301 | / | / | / | 0.983 | 65.095 |
| 40 | 8.851 | 20.13 | 0.3 | 0.17 | 0.99 | 0.81 | 0.31 | 0 | 0.251 | / | 0.04 | 0.07 | 0.983 | 67.095 |
| 41 | 8.852 | 20.16 | 0.3 | 0.72 | 0.98 | 0.91 | 0.31 | 0 | 0.252 | / | 0.07 | 0.03 | 0.989 | 66.427 |
| 42 | 6.853 | 24.152 | / | / | 1.02 | 0.91 | 0.38 | 0 | 0.251 | / | 0.03 | 0.06 | 0.984 | 65.36 |
| 43 | 5.853 | 25.152 | 0.312 | 1.12 | / | 0.51 | 0.03 | / | / | / | / | / | 0.984 | 66.039 |
| 44 | 8.846 | 22.155 | 0.2 | 1.32 | / | 1.18 | / | 0.11 | / | / | / | / | 0.985 | 65.204 |
| 45 | 5.853 | 25.153 | / | 1.02 | / | 0.19 | 0.07 | / | / | / | / | / | 0.988 | 66.726 |
| 46 | 5.852 | 25.151 | / | 1.04 | / | 0.09 | 0.09 | / | / | / | / | / | 0.983 | 66.794 |
| 47 | 14.851 | 15.153 | / | / | / | 0.91 | 0.22 | / | / | / | / | / | 0.983 | 67.883 |
| 48 | 21.152 | 8.852 | / | / | / | 0.93 | 0.21 | / | / | / | / | / | 0.989 | 67.867 |

(3) FE-EPMA inspection: the magnet material of Example 10 was taken to be polished on the vertically oriented surface, and inspected by using the Field Emission Electron Probe Microanalyser (FE-EPMA) (Japan Electronics Company (JEOL), 8530F). The distribution of elements such as Pr, Cu, B, Fe, Co and O in the magnet was first determined by FE-EPMA surface scanning, and then the content of Pr, Cu, O and other elements in the key phase was determined by FE-EPMA single point quantitative analysis, the test conditions were accelerating voltage of 15kv and probe beam current of 50nA.

The magnetic steel prepared by the formulation of the present invention was analyzed by means of the Field Emission Electron Probe Microanalyser (FE-EPMA), mainly for the elements Pr, Nd, Cu, Ti, Co and O, as shown in Figure 1, and quantitative analysis was carried out for the elements at grain boundaries and in the intergranular triangle. Wherein: the grain boundary referred to the boundary between two grains, and the intergranular triangle referred to the gap formed by three and more grains.

Figure 2 shows the distribution of elements at the grain boundaries of the neodymium-iron-boron magnet material in Example 10, Pr, Nd elements were mainly distributed in the main phase, part of the rare earth was also present at the grain boundary, element Cu and element Zr were distributed at the grain boundaries, and the point marked 1 in Figure 2 was taken for quantitative analysis of the elements at the grain boundaries, the results were shown in Table 4 below.

**Table 4**

| Pr (wt. %) | Nd (wt. %) | Cu (wt. %) | Zr (wt. %) | O (wt. %) | Fe (wt. %) |
|---|---|---|---|---|---|
| 65.2 | 12.5 | 28.6 | 0.05 | 0.79 | Residual |

From the above data, it can been seen that Pr and Nd were present at the grain boundary in the form of rare earth rich phases and oxides, which were respectively α-Pr and α-Nd, Pr₂O₃, Nd₂O₃ and NdO, and Cu occupied a certain content of about 28 wt.% at the grain boundary in addition to the main phase, for example 28.6 wt.% in this embodiment. Zr as a high melting point element was diffusely distributed throughout the region, with the effective distribution of Cu, combined with the combined effect of Pr, improved the wettability of the grain boundary, repaired crystal defects and improved the performance of the magnet.

Figure 3 shows the distribution of elements in the intergranular triangle of the neodymium-iron-boron magnet material in Example 10, the point marked 1 in Figure 3 was taken for quantitative analysis of the elements in the intergranular triangle , the results were shown in Table 5 below.

**Table 5**

| Pr (wt. %) | Nd (wt. %) | Cu (wt. %) | Zr (wt. %) | O (wt. %) | Fe (wt. %) |
|---|---|---|---|---|---|
| 42.2 | 23 | 31 | 0.02 | 1.3 | Residual |

In the intergranular triangle, Pr and Nd elements were distributed therein. In the high-Pr formulation, it is clear that Pr and Nd will be also enriched in the intergranular triangle, where the oxygen content was slightly higher than the grain boundary and the oxides formed increased, and the rare earth oxides were also distributed at the grain boundary after the ageing treatment, which was beneficial to isolate the exchange coupling among the main phases, and the magnetic properties of the magnets were ultimately improved.

## Claims

1. A raw material composition of neodymium-iron-boron magnet material, wherein, the raw material composition of neodymium-iron-boron magnet material comprises the following components by mass percentage, wherein the percentage refers to the mass percentage relative to the total mass of the raw material composition of neodymium-iron-boron magnet material: 29.5-32% of R', R' is a rare earth element and includes Pr and Nd; wherein, Pr ≥17.15%;
Cu ≥ 0.35%;
64-69.2% of Fe;
**characterized by**
0.9-1.2% of B.

2. The raw material composition according to claim 1, wherein, the content of Pr is 17.15-26%, preferably 17.15%, 18.15%, 19.15%, 20.15%, 20.85%, 21.15%, 22.15%, 23.15%, 24.15%, 25.15% or 26%;
and/or, the content of Nd is 15% or less, preferably 4-13%, more preferably 4%, 5.85%, 6.85%, 7.85%, 8.85%, 9.85%, 10.65%, 10.85%, 11.35%, 12.35% or 12.85%;
and/or, R' further comprises other rare earth elements besides Pr and Nd, preferably Y;
and/or, R' further comprises RH, RH is heavy rare earth element, the kind of RH preferably comprises one or more of Dy, Tb and Ho, more preferably Dy and/or Tb; the mass ratio of RH and R' is preferably less than 0.253, more preferably 0-0.07; wherein, the content of RH is preferably 1-2.5%, more preferably 1%, 1.5% or 2%; when RH comprises Tb, the content of Tb is preferably 0.5-2%, more preferably 0.7%, 0.8%, 0.9%, 1%, 1.5%, 1.8%, 1.9% or 2%; when RH comprises Dy, the content of Dy is preferably 1% or less, more preferably 0.1%, 0.2% or 0.3%; when RH comprises Ho, the content of Ho is preferably 0.8-2%.
and/or, the content of Cu is 0.35-1.3%, preferably 0.35%, 0.4%, 0.45%, 0.5%, 0.6%, 0.65%, 0.7%, 0.8%, 0.85%, 0.9%, 0.95%, 1%, 1.05%, 1.1% or 1.2%;
and/or, the content of B is 0.95-1.2%, preferably 0.985%, 1%, 1.1%, 1.2%;
and/or, the content of Fe is 64.8-69.2%, preferably 64.914%, 64.965%, 65.065%, 65.085%, 65.135%, 65.365%, 65.405%, 65.485%, 65.54%, 65.615%, 65.665%, 65.715%, 65.815%, 65.865%, 65.915%, 66.015%, 66.035%, 66.045%, 66.215%, 66.23%, 66.265%, 66.315%, 66.465%, 66.445%, 66.545%, 66.615%, 66.715%, 66.815%, 66.865%, 67.145%, 67.165%, 67.415%, 67.615%, 67.915%, 68.015%, 68.295%, 68.565% or 69.165%;
and/or, the raw material composition of neodymium-iron-boron magnet material further comprises Al; preferably, the content of Al is 3% or less, preferably 0.5% or less, more preferably 0.02%, 0.03%, 0.1%, 0.2%, 0.25%, 0.3%, 0.4%, 0.45%, 0.46% or 0.48%;
and/or, the raw material composition of neodymium-iron-boron magnet material further comprises Ga; preferably, the content of Ga is 1% or less, preferably 0.05-0.6%, more preferably 0.1%, 0.15%, 0.18%, 0.2%, 0.24%, 0.25%, 0.3%, 0.4% or 0.5%;
and/or, the raw material composition of neodymium-iron-boron magnet material further comprises Zr; preferably, the content of Zr is 0.3% or less, preferably 0.1%, 0.2%, 0.22%, 0.25%, 0.26%, 0.27%, 0.28%, 0.29% or 0.3%;
and/or, the raw material composition of neodymium-iron-boron magnet material further comprises Co; preferably, the content of Co is 0.2-1.5%, preferably 0.2% or 1%;
and/or, the raw material composition of neodymium-iron-boron magnet material may further comprise one or more of Zn, Ag, In, Sn, V, Cr, Mo, Ta, Hf and W; wherein, preferably, the content of Zn is 0.1% or less, preferably 0.04-0.08%, better 0.04%, 0.05% or 0.08%; wherein, preferably, the content of Mo is 0.1% or less, preferably 0.01-0.08%, more preferably 0.04%, 0.05% or 0.08%.

3. The raw material composition according to claim 1 or 2, wherein, the raw material composition comprises the following components by mass percentage: 29.5-32% of R', R' is a rare earth element and comprises Pr and Nd; wherein, Pr ≥17.15%; Cu ≥0.35%; Al≤0.5%; 0.25-0.3% of Zr; 0.9-1.2% of B; 64-69.2% of Fe;
preferably, the content of Pr is 17.15-26%; preferably, the content of Cu is 0.35-1.2%; preferably, R' further comprises RH, RH is a heavy rare earth element, the content of the heavy rare earth element is preferably 1-2.5%; the kind of RH preferably comprises Dy and/or Tb, wherein, the content of Tb is preferably 0.5-2%, the content of Dy is preferably 1% or less; the percentage refers to the mass percentage relative to the total mass of the raw material composition of neodymium-iron-boron magnet material.

4. The raw material composition according to claim 1 or 2, wherein, the raw material composition comprises the following components by mass percentage: 29.5-32% of R', R' is a rare earth element and comprises Pr and Nd; wherein, Pr ≥17.15%; Cu ≥0.35%; Al≤0.5%; Ga≤0.42%; 0.25-0.3% of Zr; 0.9-1.2% of B; 64-69.2% of Fe;
preferably, the content of Pr is 17.15-26%; preferably, the content of Cu is 0.35-1.2%; preferably, R' comprises RH, RH is a heavy rare earth element, the content of the heavy rare earth element is preferably 1-2.5%; the kind of RH preferably comprises Dy and/or Tb, wherein, the content of Tb is preferably 0.5-2%, the content of Dy is preferably 1% or less; the percentage refers to the mass percentage relative to the total mass of the raw material composition of neodymium-iron-boron magnet material.

5. A preparation method for neodymium-iron-boron magnet material, wherein, the neodymium-iron-boron magnet material is prepared by using the raw material composition according to any one of claims 1-4;
preferably, the preparation method comprises the following steps: the molten liquid of the raw material composition according to any one of claims 1 to 4 is subjected to melting and casting, hydrogen decrepitation, forming, sintering and ageing treatment;
more preferably, after sintering and before the ageing treatment, a grain boundary diffusion treatment is further carried out.

6. A neodymium-iron-boron magnet material, wherein, the neodymium-iron-boron magnet material comprises the following components by mass percentage, wherein the percentage refers to the mass percentage relative to the total mass of the raw material composition of neodymium-iron-boron magnet material: 29.4-32.6% of R', R' comprises Pr and Nd; wherein, Pr ≥17.14%;
Cu >_ 0.34%;
64-69.2% of Fe;
**characterized by**
0.9-1.2% of B.

7. The neodymium-iron-boron magnet material according to claim 6, wherein, the content of Pr is 17.14-26.1%, preferably 17.149%, 17.15%, 17.154%, 18.15%, 18.152%, 18.154%, 18.155%, 19.15%, 19.152%, 19.154%, 19.155%, 19.159%, 20.13%, 20.155%, 20.16%, 21.157%, 22.15%, 22.151%, 22.152%, 22.1555%, 23.15%, 24.151%, 24.152%, 24.155%, 24.157%, 24.158%, 25.15%, 25.152%, 25.153%, 25.156% or 26.01%;
and/or, the content of Nd is 15% or less, preferably 4-13%, more preferably 4.02%, 5.847%, 5.84%, 5.849%, 5.85%, 5.851%, 5.852%, 5.853%, 5.854%, 6.851%, 6.852%, 6.853%, 7.85%, 8.846%, 8.847%, 8.85%, 8.851%, 8.852%, 8.853%, 9.85%, 9.851%, 10.844%, 10.846%, 10.849%, 11.349%, 11.384%, 12.341%, 12.345%, 12.348%, 12.35%, 12.351% ,12.364%, 12.791%, 12.802% or 12.849%;
and/or, the ratio of the mass of Nd to the total mass of R' is less than 0.5, preferably 0.1-0.45;
and/or, the content of R' is preferably 29.49-32.53%, more preferably 29.495%, 29.501%, 30.003%, 30.004%, 30.03%, 30.441%, 30.517%, 30.518%, 30.957%, 30.98%, 31%, 31.006%, 31.0065%, 31.009%, 31.011%, 31.012%, 31.013%, 31.498%, 31.504%, 31.539%, 31.946%, 31.972%, 31.977%, 31.995%, 31.999%, 32%, 32.001%, 32.013%, 32.015%, 32.021%, 32.022%, 32.023%, 32.024%, 32.025%, 32.026%, 32.027%, 32.04%, 32.043%, 32.437% or 32.521%;
and/or, R' further comprises other rare earth elements besides Pr and Nd, preferably Y;
and/or, R' further comprises RH, RH is a heavy rare earth element, the kind of RH preferably comprises one or more of Dy, Tb and Ho, more preferably Dy and/or Tb; preferably, the mass ratio of RH and R' is preferably less than 0.253, preferably 0-0.07, more preferably 1.01/32.015, 1.02/30.517, 1.02/32.021, 1.02/32.023, 1.02/32.024, 1.02/32.024, 1.02/32.025, 1.02/32.025, 1.02/32.026, 1.03/32.04, 1.04/32.043, 1.432/32.437, 1.46/30.441, 1.47/31.972, 1.48/31.977, 1.5/32, 1.52/32.521, 1.98/30.98, 1.99/31.995, 1/31.999, 1/32, 2.01/31.011, 2.01/31.013, 2.01/32.013, 2.02/32.022, 2.02/32.027, 2/31 or 2/31.012; wherein, the content of RH is preferably 1-2.5%, more preferably 1%, 1.01%, 1.02%, 1.03%, 1.04%, 1.432%, 1.46%, 1.47%, 1.48%, 1.5%, 1.52%, 1.98%, 1.99%, 2%, 2.01% or 2.02%; wherein, when RH comprises Tb, the content of Tb is preferably 0.5-2wt.%, more preferably 0.7%, 0.72%, 0.82%, 0.9%, 0.91%, 1%, 1.02%, 1.47%, 1.48%, 1.5%, 1.81%, 1.88%, 1.89%, 1.9%, 1.91% or 2.01%; when RH comprises Dy, the content of Dy is preferably 0.5wt.% or less, more preferably 0.1%, 0.2%, 0.21%, 0.3%, 0.31% or 0.312%; when RH comprises Ho, the content of Ho is preferably 0.8-2%, more preferably 0.98%, 0.99% or 1%;
and/or, the content of Cu is 0.34-1.3%, preferably 0.341%, 0.41%, 0.452%, 0.47%, 0.502%, 0.51%, 0.52%, 0.598%, 0.62%, 0.648%, 0.649%, 0.701%, 0.702%, 0.71%, 0.78%, 0.79%, 0.795%, 0.806%, 0.81%, 0.852%, 0.89%, 0.901%, 0.903%, 0.91%, 0.92%, 0.948%, 1.021%, 1.05%, 1.08%, 1.101%, 1.103%, 1.12%, 1.18%, 1.19%, 1.202% or 1.21%;
and/or, the content of B is 0.95-1.2%, preferably 0.983%, 0.984%, 0.985%, 0.988%, 0.989%, 1.02% or 1.19%;
and/or, the content of Fe is 64.8-69.2%, preferably 64.965% ,65.031%, 65.095%, 65.155%, 65.204%, 65.36%, 65.4%, 65.458%, 65.525%, 65.626%, 65.63%, 65.686%, 65.817%, 65.8395%, 65.869%, 65.909%, 65.963%, 65.994%, 65.995%, 66.039%, 66.04%, 66.099%, 66.157%, 66.218%, 66.267%, 66.364%, 66.377%, 66.427%, 66.437%, 66.52%, 66.605%, 66.671%, 66.8075%, 66.81%, 66.87%, 67.095%, 67.12%, 67.137%, 67.457%, 67.578%, 67.996%, 68.302%, 68.556% or 69.181%; and/or, the neodymium-iron-boron magnet material further comprises Al; preferably, the content of Al is 0.5% or less, preferably 0.03-0.5wt.%, more preferably 0.01%, 0.02%, 0.03%, 0.1%, 0.102%, 0.12%, 0.2%, 0.21%, 0.24%, 0.25%, 0.29%, 0.3%, 0.31%, 0.38%, 0.4%, 0.42%, 0.45%, 0.46% or 0.48%;
and/or, the neodymium-iron-boron magnet material further comprises Zr; preferably, the content of Zr is 0.05-0.31wt.% by weight, preferably 0.1%, 0.21%, 0.22%, 0.25%, 0.251%, 0.252%, 0.261%, 0.272%, 0.28%, 0.281%, 0.282%, 0.291% 0.3% or 0.301%;
and/or, the neodymium-iron-boron magnet material further comprises Ga; preferably, the content of Ga is 0.51% or less, preferably 0.1-0.51%, more preferably 0.1%, 0.101%, 0.102%, 0.11%, 0.12%, 0.152%, 0.18%, 0.2%, 0.202%, 0.24%, 0.25%, 0.251%, 0.302%, 0.401% or 0.501%;
and/or, the neodymium-iron-boron magnet material further comprises Co; preferably, the content of Co is 0.2-1.5%, preferably 0.2% or 1%;
and/or, the neodymium-iron-boron magnet material further comprises O; preferably, the content of O is 0.13% or less;
and/or, the neodymium-iron-boron magnet material may further comprise one or more of Zn, Ag, In, Sn, V, Cr, Mo, Ta, Hf and W; wherein, the content of Zn is preferably 0.02-0.08%, more preferably 0.03%, 0.04% or 0.07%; wherein, the content of Mo is preferably 0.01-0.08%, more preferably 0.03%, 0.06% or 0.07%.

8. A neodymium-iron-boron magnet material, wherein, in the intergranular triangle region of the neodymium-iron-boron magnet material, the ratio of the total mass of Pr and Cu to the total mass of each element in the intergranular triangle region is Q1;
at the grain boundary of the neodymium-iron-boron magnet material, the ratio of the total mass of Pr and Cu to the total mass of each element at the grain boundary is Q2;
wherein, Q1 < Q2, and Q2 ≥ 0.1; and
wherein the components of the neodymium-iron-boron magnet material refer to the neodymium-iron-boron magnet material according to any one of claims 6-7.

9. An application of the neodymium-iron-boron magnet material according to any one of claims 6-8 as an electronic component in a motor.

## Patentansprüche

1. Eine Rohmaterialzusammensetzung eines Neodym-Eisen-Bor-Magnetmaterials, wobei die Rohmaterialzusammensetzung des Neodym-Eisen-Bor-Magnetmaterials die folgenden Komponenten in Massenprozent umfasst, wobei sich der Prozentsatz auf den Massenprozentsatz relativ zur Gesamtmasse der Rohmaterialzusammensetzung des Neodym-Eisen-Bor-Magnetmaterials bezieht:
29,5-32% R', R' ist ein Seltenerdelement und umfasst Pr und Nd; wobei Pr
≥17,15%;
Cu ≥ 0,35%;
64-69,2% Fe;
**gekennzeichnet durch**
0,9-1,2% B.

2. Rohmaterialzusammensetzung nach Anspruch 1, wobei der Gehalt von Pr 17,15-26%, vorzugsweise 17,15%, 18,15%, 19,15%, 20,15%, 20,85%, 21,15%, 22,15%, 23,15%, 24,15%, 25,15% oder 26% beträgt;
und/oder der Gehalt von Nd beträgt 15% oder weniger, vorzugsweise 4-13%, mehr bevorzugt 4%, 5,85%, 6,85%, 7,85%, 8,85%, 9,85%, 10,65%, 10,85%, 11,35%, 12,35% oder 12,85%;
und/oder R' umfasst weiterhin andere Seltenerdelemente neben Pr und Nd, vorzugsweise Y;
und/oder R' umfasst weiterhin RH, RH ist ein schweres Seltenerdelement, die Art von RH umfasst vorzugsweise eines oder mehrere von Dy, Tb und Ho, vorzugsweise Dy und/oder Tb; das Massenverhältnis von RH und R' beträgt vorzugsweise weniger als 0,253, vorzugsweise 0-0,07; wobei der Gehalt von RH vorzugsweise 1-2,5%, mehr bevorzugt 1%, 1,5% oder 2% beträgt; wenn RH Tb umfasst, beträgt der Gehalt von Tb vorzugsweise 0,5-2%, mehr bevorzugt 0,7%, 0,8%, 0,9%, 1%, 1,5%, 1,8%, 1,9% oder 2%; wenn RH Dy umfasst, beträgt der Gehalt von Dy vorzugsweise 1% oder weniger, mehr bevorzugt 0,1%, 0,2% oder 0,3%; wenn RH Ho umfasst, beträgt der Gehalt von Ho vorzugsweise 0,8-2%;
und/oder der Gehalt von Cu beträgt 0,35-1,3%, vorzugsweise 0,35%, 0,4%, 0,45%, 0,5%, 0,6%, 0,65%, 0,7%, 0,8%, 0,85%, 0,9%, 0,95%, 1%, 1,05%, 1,1% oder 1,2%; und/oder der Gehalt von B beträgt 0,95-1,2%, vorzugsweise 0,985%, 1%, 1,1%, 1,2%;
und/oder der Gehalt von Fe beträgt 64,8-69,2%, vorzugsweise 64,914%, 64,965%, 65,065%, 65,085%, 65,135%, 65,365%, 65,405%, 65,485%, 65,54%, 65,615%, 65,665%, 65,715%, 65,815%, 65,865%, 65,915%, 66,015%, 66. 035%, 66,045%, 66,215%, 66,23%, 66,265%, 66,315%, 66,465%, 66,445%, 66,545%, 66,615%, 66,715%, 66,815%, 66,865%, 67,145%, 67,165%, 67,415%, 67,615%, 67,915%, 68,015%, 68,295%, 68,565% oder 69,165%;
und/oder die Rohmaterialzusammensetzung des Neodym-Eisen-Bor-Magnetmaterials umfasst weiterhin Al; vorzugsweise beträgt der Gehalt von Al 3% oder weniger, vorzugsweise 0,5% oder weniger, mehr bevorzugt 0,02%, 0,03%, 0,1%, 0,2%, 0,25%, 0,3%, 0,4%, 0,45%, 0,46% oder 0,48%;
und/oder die Rohmaterialzusammensetzung des Neodym-Eisen-Bor-Magnetmaterials umfasst weiterhin Ga; vorzugsweise beträgt der Gehalt von Ga 1% oder weniger, vorzugsweise 0,05-0,6%, mehr bevorzugt 0,1%, 0,15%, 0,18%, 0,2%, 0,24%, 0,25%, 0,3%, 0,4% oder 0,5%;
und/oder die Rohmaterialzusammensetzung des Neodym-Eisen-Bor-Magnetmaterials umfasst weiterhin Zr; vorzugsweise beträgt der Gehalt von Zr 0,3% oder weniger, vorzugsweise 0,1%, 0,2%, 0,22%, 0,25%, 0,26%, 0,27%, 0,28%, 0,29% oder 0,3%;
und/oder die Rohmaterialzusammensetzung des Neodym-Eisen-Bor-Magnetmaterials umfasst weiterhin Co; vorzugsweise beträgt der Gehalt von Co 0,2-1,5%, vorzugsweise 0,2% oder 1%;
und/oder die Rohmaterialzusammensetzung des Neodym-Eisen-Bor-Magnetmaterials kann weiterhin eines oder mehrere der Elemente Zn, Ag, In, Sn, V, Cr, Mo, Ta, Hf und W umfassen; wobei der Gehalt von Zn vorzugsweise 0,1% oder weniger, vorzugsweise 0,04-0,08%, besser 0,04%, 0,05% oder 0,08% beträgt; wobei der Gehalt von Mo vorzugsweise 0,1% oder weniger, vorzugsweise 0,01-0,08%, besser 0,04%, 0,05% oder 0,08% beträgt.

3. Rohmaterialzusammensetzung nach Anspruch 1 oder 2, wobei die Rohmaterialzusammensetzung die folgenden Komponenten in Massenprozent umfasst: 29,5-32% R', R' ist ein Seltenerdelement und umfasst Pr und Nd; wobei Pr ≥17,15%; Cu ≥0,35%; Al≤0,5%; 0,25-0,3% Zr; 0,9-1,2% B; 64-69,2% Fe; vorzugsweise beträgt der Gehalt von Pr 17,15-26%; vorzugsweise beträgt der Gehalt von Cu 0,35-1,2%; vorzugsweise umfasst R' ferner RH, RH ist ein schweres Seltenerdelement, der Gehalt des schweren Seltenerdelements beträgt vorzugsweise 1-2,5%; die Art von RH umfasst vorzugsweise Dy und/oder Tb, wobei der Gehalt von Tb vorzugsweise 0,5-2% beträgt, der Gehalt von Dy vorzugsweise 1% oder weniger beträgt; der Prozentsatz bezieht sich auf den Massenprozentsatz relativ zur Gesamtmasse der Rohmaterialzusammensetzung des Neodym-Eisen-Bor-Magnetmaterials.

4. Rohmaterialzusammensetzung nach Anspruch 1 oder 2, wobei die Rohmaterialzusammensetzung die folgenden Komponenten in Massenprozent umfasst: 29,5-32% R', R' ist ein Seltenerdelement und umfasst Pr und Nd; wobei Pr ≥17,15%; Cu ≥0,35%; Al≤0,5%; Ga≤0,42%; 0,25-0,3% Zr; 0,9-1,2% B; 64-69,2% Fe;
vorzugsweise beträgt der Gehalt von Pr 17,15-26%; vorzugsweise beträgt der Gehalt von Cu 0,35-1,2%; vorzugsweise umfasst R' RH, RH ist ein schweres Seltenerdelement, der Gehalt des schweren Seltenerdelements beträgt vorzugsweise 1-2,5%; die Art von RH umfasst vorzugsweise Dy und/oder Tb, wobei der Gehalt von Tb vorzugsweise 0,5-2% beträgt, der Gehalt von Dy vorzugsweise 1% oder weniger beträgt; der Prozentsatz bezieht sich auf den Massenprozentsatz relativ zur Gesamtmasse der Rohmaterialzusammensetzung des Neodym-Eisen-Bor-Magnetmaterials.

5. Ein Herstellungsverfahren für Neodym-Eisen-Bor-Magnetmaterial, wobei das Neodym-Eisen-Bor-Magnetmaterial unter Verwendung der Rohmaterialzusammensetzung nach einem der Ansprüche 1 bis 4 hergestellt wird; vorzugsweise umfasst das Herstellungsverfahren die folgenden Schritte: Die geschmolzene Flüssigkeit der Rohstoffzusammensetzung nach einem der Ansprüche 1 bis 4 wird einem Schmelz- und Gießvorgang, einr Wasserstoffdekrepitation, Formgebung, Sinterung und Alterungsbehandlung unterzogen;
mehr bevorzugt wird nach dem Sintern und vor der Alterungsbehandlung eine Korngrenzendiffusionsbehandlung durchgeführt.

6. Neodym-Eisen-Bor-Magnetmaterial, wobei das Neodym-Eisen-Bor-Magnetmaterial die folgenden Komponenten in Massenprozent umfasst, wobei sich der Prozentsatz auf den Massenprozentsatz relativ zur Gesamtmasse der Rohmaterialzusammensetzung des Neodym-Eisen-Bor-Magnetmaterials bezieht:
29,4-32,6% R', wobei R' Pr und Nd umfasst; wobei Pr ≥17,14%;
Cu ≥ 0,34%;
64-69,2% Fe;
**gekennzeichnet durch**
0,9-1,2% B.

7. Neodym-Eisen-Bor-Magnetmaterial nach Anspruch 6, wobei der Gehalt von Pr 17,14-26,1%, vorzugsweise 17,149%, 17,15%, 17,154%, 18,15%, 18,152%, 18,154%, 18,155%, 19,15%, 19,152%, 19,154%, 19,155%, 19,159%, 20,13%, 20,155%, 20,16%, 21,157%, 22,15%, 22,151%, 22,152%, 22,1555%, 23,15%, 24,151%, 24,152%, 24,155%, 24,157%, 24,158%, 25,15%, 25,152%, 25,153%, 25,156% oder 26,01% beträgt;
und/oder der Gehalt von Nd beträgt 15% oder weniger, vorzugsweise 4-13%, mehr bevorzugt 4,02%, 5,847%, 5,84%, 5,849%, 5,85%, 5,851%, 5,852%, 5,853%, 5,854%, 6,851%, 6,852%, 6,853%, 7,85%, 8,846%, 8,847%, 8,85%, 8,851%, 8,852%, 8,853%, 9,85%, 9,851%, 10,844%, 10,846%, 10,849%, 11,349%, 11,384%, 12,341%, 12,345%, 12,348%, 12,35%, 12,351%, 12,364%, 12,791%, 12,802% oder 12,849%;
und/oder das Verhältnis der Masse von Nd zur Gesamtmasse von R' beträgt weniger als 0,5, vorzugsweise 0,1-0,45;
und/oder der Gehalt von R' beträgt vorzugsweise 29,49-32,53%, mehr bevorzugt 29,495%, 29,501%, 30,003%, 30,004%, 30,03%, 30,441%, 30,517%, 30,518%, 30,957%, 30,98%, 31%, 31,006%, 31,0065%, 31,009%, 31,011%, 31,012%, 31,013%, 31,498%, 31,504%, 31,539%, 31,946%, 31,972%, 31,977%, 31,995%, 31,999%, 32%, 32,001%, 32,013%, 32,015%, 32,021%, 32,022%, 32,023%, 32,024%, 32,025%, 32,026%, 32,027%, 32,04%, 32,043%, 32,437% oder 32,521%; und/oder umfasst R' außerdem andere Seltenerdelemente neben Pr und Nd, vorzugsweise Y;
und/oder R' umfasst weiterhin RH, RH ist ein schweres Seltenerdelement, die Art von RH umfasst vorzugsweise eines oder mehrere von Dy, Tb und Ho, mehr bevorzugt Dy und/oder Tb; vorzugsweise ist das Massenverhältnis von RH zu R' kleiner als 0,253, vorzugsweise 0-0,07, mehr bevorzugt 1,01/32,015, 1,02/30,517, 1,02/32,021, 1,02/32,023, 1,02/32,024, 1,02/32,024, 1,02/32,025, 1,02/32,025, 1,02/32,026, 1,03/32,04, 1,04/32,043, 1,432/32,437, 1,46/30,441, 1,47/31,972, 1,48/31,977, 1,5/32, 1,52/32,521, 1,98/30,98, 1,99/31,995, 1/31,999, 1/32, 2,01/31,011, 2,01/31,013, 2,01/32,013, 2,02/32,022, 2,02/32,027, 2/31 oder 2131,012; wobei der Gehalt von RH vorzugsweise 1-2,5 %, mehr bevorzugt 1%, 1,01%, 1,02%, 1,03%, 1,04%, 1,432%, 1,46%, 1,47%, 1,48%, 1,5%, 1,52%, 1,98%, 1,99%, 2%, 2,01% oder 2,02% beträgt; wobei, wenn RH Tb umfasst, der Gehalt von Tb vorzugsweise 0,5-2 Gew.-%, mehr bevorzugt 0,7%, 0,72%, 0,82%, 0,9%, 0,91%, 1%, 1,02%, 1,47%, 1,48%, 1,5%, 1,81%, 1,88%, 1,89%, 1,9%, 1,91% oder 2,01% beträgt; wenn RH Dy umfasst, beträgt der Gehalt von Dy vorzugsweise 0,5 Gew.-% oder weniger, mehr bevorzugt 0,1%, 0,2%, 0,21%, 0,3%, 0,31% oder 0,312%; wenn RH Ho umfasst, beträgt der Gehalt von Ho vorzugsweise 0,8-2%, mehr bevorzugt 0,98%, 0,99% oder 1%;
und/oder der Gehalt von Cu beträgt 0,34-1,3%, vorzugsweise 0,341%, 0,41%, 0,452%, 0,47%, 0,502%, 0,51%, 0,52%, 0,598%, 0,62%, 0,648%, 0,649%, 0,701%, 0,702%, 0,71%, 0,78%, 0,79%, 0,795%, 0,806%, 0,81%, 0,852%, 0,89%, 0,901%, 0,903%, 0,91%, 0,92%, 0,948%, 1,021%, 1,05%, 1,08%, 1,101%, 1,103%, 1,12%, 1,18%, 1,19%, 1,202% oder 1,21%;
und/oder der Gehalt von B beträgt 0,95-1,2%, vorzugsweise 0,983%, 0,984%, 0,985%, 0,988%, 0,989%, 1,02% oder 1,19%;
und/oder der Gehalt von Fe beträgt 64,8-69,2%, vorzugsweise 64,965%, 65,031%, 65,095%, 65,155%, 65,204%, 65,36%, 65,4%, 65,458%, 65,525%, 65,626%, 65,63%, 65,686%, 65,817%, 65,8395%, 65,869%, 65,909%, 65,963%, 65,994%, 65,995%, 66,039%, 66,04%, 66,099%, 66,157%, 66,218%, 66,267%, 66,364%, 66,377%, 66,427%, 66,437%, 66,52%, 66,605%, 66,671%, 66,8075%, 66,81%, 66,87%, 67,095%, 67,12%, 67,137%, 67,457%, 67,578%, 67,996%, 68,302%, 68,556% oder 69,181%;
und/oder das Neodym-Eisen-Bor-Magnetmaterial umfasst weiterhin Al; vorzugsweise beträgt der Gehalt von Al 0,5% oder weniger, vorzugsweise 0,03-0,5 Gew.-%, mehr bevorzugt 0,01%, 0,02%, 0,03%, 0,1%, 0,102%, 0,12%, 0,2%, 0,21%, 0,24%, 0,25%, 0,29%, 0,3%, 0,31%, 0,38%, 0,4%, 0,42%, 0,45%, 0,46% oder 0,48%;
und/oder das Neodym-Eisen-Bor-Magnetmaterial umfasst weiterhin Zr; vorzugsweise beträgt der Gehalt von Zr 0,05-0,31 Gew.-%, vorzugsweise 0,1%, 0,21%, 0,22%, 0,25%, 0,251%, 0,252%, 0,261%, 0,272%, 0,28%, 0,281%, 0,282%, 0,291%, 0,3% oder 0,301%;
und/oder das Neodym-Eisen-Bor-Magnetmaterial umfasst weiterhin Ga; vorzugsweise beträgt der Gehalt von Ga 0,51% oder weniger, vorzugsweise 0,1-0,51%, mehr bevorzugt 0,1%, 0,101%, 0,102%, 0,11%, 0,12%, 0,152%, 0,18%, 0,2%, 0,202%, 0,24%, 0,25%, 0,251%, 0,302%, 0,401% oder 0,501%;
und/oder das Neodym-Eisen-Bor-Magnetmaterial umfasst weiterhin Co; vorzugsweise beträgt der Gehalt von Co 0,2-1,5%, vorzugsweise 0,2% oder 1%;
und/oder das Neodym-Eisen-Bor-Magnetmaterial umfasst weiterhin O; vorzugsweise beträgt der O-Gehalt 0,13% oder weniger;
und/oder das Neodym-Eisen-Bor-Magnetmaterial kann weiterhin eines oder mehrere der Elemente Zn, Ag, In, Sn, V, Cr, Mo, Ta, Hf und W umfassen, wobei der Gehalt von Zn vorzugsweise 0,02 bis 0,08%, mehr bevorzugt 0,03%, 0,04% oder 0,07% beträgt; wobei der Gehalt von Mo vorzugsweise 0,01 bis 0,08%, mehr bevorzugt 0,03%, 0,06% oder 0,07% beträgt.

8. Neodym-Eisen-Bor-Magnetmaterial, wobei in dem intergranularen Dreiecksbereich des Neodym-Eisen-Bor-Magnetmaterials das Verhältnis der Gesamtmasse von Pr und Cu zu der Gesamtmasse jedes Elements in dem intergranularen Dreiecksbereich Q1 ist;
an der Korngrenze des Neodym-Eisen-Bor-Magnetmaterials das Verhältnis der Gesamtmasse von Pr und Cu zu der Gesamtmasse jedes Elements an der Korngrenze Q2 ist;
wobei Q1 < Q2, und Q2 ≥ 0,1 ist; und
wobei sich die Komponenten des Neodym-Eisen-Bor-Magnetmaterials auf das Neodym-Eisen-Bor-Magnetmaterial nach einem der Ansprüche 6-7 beziehen.

9. Verwendung des Neodym-Eisen-Bor-Magnetmaterials nach einem der Ansprüche 6-8 als elektronische Komponente in einem Motor.

## Revendications

1. Composition de matière première de matériau magnétique de néodyme-fer-bore, la composition de matière première de matériau magnétique de néodyme-fer-bore comprenant les composants suivants en pourcentage en masse, le pourcentage faisant référence au pourcentage en masse par rapport à la masse totale de la composition de matière première de matériau magnétique de néodyme-fer-bore :
29,5-32 % de R', R' étant un élément des terres rares et comprenant Pr et Nd ;
Pr ≥ 17,15 % ;
Cu ≥ 0,35 % ;
64-69,2 % de Fe ;
**caractérisée par**
0,9-1,2 % de B.

2. Composition de matière première selon la revendication 1, la teneur de Pr étant 17,15-26 %, préférablement 17,15 %, 18,15 %, 19,15 %, 20,15 %, 20,85 %, 21,15 %, 22,15 %, 23,15 %, 24,15 %, 25,15 % ou 26 % ;
et/ou, la teneur de Nd étant 15 % ou moins, préférablement 4-13 %, plus préférablement 4 %, 5,85 %, 6,85 %, 7,85 %, 8,85 %, 9,85 %, 10,65 %, 10,85 %, 11,35 %, 12,35 % ou 12,85 % ;
et/ou, R' comprenant en outre d'autres éléments des terres rares outre Pr et Nd, préférablement Y ;
et/ou, R' comprenant en outre RH, RH étant un élément lourd des terres rares, la sorte de RH préférablement comprenant un ou plusieurs parmi Dy, Tb et Ho, plus préférablement Dy et/ou Tb ; le rapport en masse de RH et R' étant préférablement inférieur à 0,253, plus préférablement 0-0,07 ; la teneur de RH étant préférablement 1-2,5 %, plus préférablement 1 %, 1,5 % ou 2 % ; lorsque RH comprend Tb, la teneur de Tb étant préférablement 0,5-2 %, plus préférablement 0,7 %, 0,8 %, 0,9 %, 1 %, 1,5 %, 1,8 %, 1,9 % ou 2 % ; lorsque RH comprend Dy, la teneur de Dy étant préférablement 1 % ou moins, plus préférablement 0,1 %, 0,2 % ou 0,3 % ; lorsque RH comprend Ho, la teneur de Ho étant préférablement 0,8-2 %, et/ou, la teneur de Cu étant 0,35-1,3 %, préférablement 0,35 %, 0,4 %, 0,45 %, 0,5 %, 0,6 %, 0,65 %, 0,7 %, 0,8 %, 0,85 %, 0,9 %, 0,95 %, 1 %, 1,05 %, 1,1 % ou 1,2 % ;
et/ou, la teneur de B étant 0,95-1,2 %, préférablement 0,985 %, 1 %, 1,1 %, 1,2 % ;
et/ou, la teneur de Fe étant 64,8-69,2 %, préférablement 64,914 %, 64,965 %, 65,065 %, 65,085 %, 65,135 %, 65,365 %, 65,405 %, 65,485 %, 65,54 %, 65,615 %, 65,665 %, 65,715 %, 65,815 %, 65,865 %, 65,915 %, 66,015 %, 66,035 %, 66,045 %, 66,215 %, 66,23 %, 66,265 %, 66,315 %, 66,465 %, 66,445 %, 66,545 %, 66,615 %, 66,715 %, 66,815 %, 66,865 %, 67,145 %, 67,165 %, 67,415 %, 67,615 %, 67,915 %, 68,015 %, 68,295 %, 68,565 % ou 69,165 % ;
et/ou, la composition de matière première de matériau magnétique de néodyme-fer-bore comprenant en outre Al ; préférablement, la teneur de Al étant 3 % ou moins, préférablement 0,5 % ou moins, plus préférablement 0,02 %, 0,03 %, 0,1 %, 0,2 %, 0,25 %, 0,3 %, 0,4 %, 0,45 %, 0,46 % ou 0,48 % ;
et/ou, la composition de matière première de matériau magnétique de néodyme-fer-bore comprenant en outre Ga ; préférablement, la teneur de Ga étant 1 % ou moins, préférablement 0,05-0,6 %, plus préférablement 0,1 %, 0,15 %, 0,18 %, 0,2 %, 0,24 %, 0,25 %, 0,3 %, 0,4 % ou 0,5 % ;
et/ou, la composition de matière première de matériau magnétique de néodyme-fer-bore comprenant en outre Zr ; préférablement, la teneur de Zr étant 0,3 % ou moins, préférablement 0,1 %, 0,2 %, 0,22 %, 0,25 %, 0,26 %, 0,27 %, 0,28 %, 0,29 % ou 0,3 % ;
et/ou, la composition de matière première de matériau magnétique de néodyme-fer-bore comprenant en outre Co ; préférablement, la teneur de Co étant 0,2-1,5 %, préférablement 0,2 % ou 1 % ;
et/ou, la composition de matière première de matériau magnétique de néodyme-fer-bore pouvant en outre comprendre un ou plusieurs parmi Zn, Ag, In, Sn, V, Cr, Mo, Ta, Hf et W ; préférablement, la teneur de Zn étant 0,1 % ou moins, préférablement 0,04-0,08 %, mieux 0,04 %, 0,05 % ou 0,08 % ; préférablement, la teneur de Mo étant 0,1 % ou moins, préférablement 0,01-0,08 %, plus préférablement 0,04 %, 0,05 % ou 0,08 %.

3. Composition de matière première selon la revendication 1 ou 2, la composition de matière première comprenant les composants suivants en pourcentage en masse : 29,5-32 % de R', R' étant un élément des terres rares et comprenant Pr et Nd ; Pr ≥ 17,15 % ; Cu ≥ 0,35 % ; Al ≤ 0,5 % ; 0,25-0,3 % de Zr ; 0,9-1,2 % de B ; 64-69,2 % de Fe ;
préférablement, la teneur de Pr étant 17,15-26 % ; préférablement, la teneur de Cu étant 0,35-1,2 % ; préférablement, R' comprenant en outre RH, RH étant un élément lourd des terres rares, la teneur de l'élément lourd des terres rares étant préférablement 1-2,5 % ; la sorte de RH préférablement comprenant Dy et/ou Tb, la teneur de Tb étant préférablement 0,5-2 %, la teneur de Dy étant préférablement 1 % ou moins ; le pourcentage faisant référence au pourcentage en masse par rapport à la masse totale de la composition de matière première de matériau magnétique de néodyme-fer-bore.

4. Composition de matière première selon la revendication 1 ou 2, la composition de matière première comprenant les composants suivants en pourcentage en masse : 29,5-32 % de R', R' étant un élément des terres rares et comprenant Pr et Nd ; Pr ≥ 17,15 % ; Cu ≥ 0,35 % ; Al ≤ 0,5 % ; Ga ≤ 0,42 % ; 0,25-0,3 % de Zr ; 0,9-1,2 % de B ; 64-69,2 % de Fe ;
préférablement, la teneur de Pr étant 17,15-26 % ; préférablement, la teneur de Cu étant 0,35-1,2 % ; préférablement, R' comprenant RH, RH étant un élément lourd des terres rares, la teneur de l'élément lourd des terres rares étant préférablement 1-2,5 % ; la sorte de RH préférablement comprenant Dy et/ou Tb, la teneur de Tb étant préférablement 0,5-2 %, la teneur de Dy étant préférablement 1 % ou moins ; le pourcentage faisant référence au pourcentage en masse par rapport à la masse totale de la composition de matière première de matériau magnétique de néodyme-fer-bore.

5. Procédé de préparation pour un matériau magnétique de néodyme-fer-bore, le matériau magnétique de néodyme-fer-bore étant préparé en utilisant la composition de matière première selon l'une quelconque des revendications 1 à 4 ; préférablement, le procédé de préparation comprenant les étapes suivantes : le liquide fondu de la composition de matière première selon l'une quelconque des revendications 1 à 4 étant soumise à une fusion et une coulée, une décrépitation par l'hydrogène, une mise en forme, un frittage et un traitement de vieillissement ; plus préférablement, après frittage et avant le traitement de vieillissement, un traitement de diffusion intragranulaire étant en outre mis en oeuvre.

6. Matériau magnétique de néodyme-fer-bore, le matériau magnétique de néodyme-fer-bore comprenant les composants suivants en pourcentage en masse, le pourcentage faisant référence au pourcentage en masse par rapport à la masse totale de la composition de matière première de matériau magnétique de néodyme-fer-bore :
29,4-32,6 % de R', R' comprenant Pr et Nd ; Pr z 17,14 % ;
Cu ≥ 0,34 % ;
64-69,2 % de Fe ;
**caractérisé par**
0,9-1,2 % de B.

7. Matériau magnétique de néodyme-fer-bore selon la revendication 6, la teneur de Pr étant 17,14-26,1 %, préférablement 17,149 %, 17,15 %, 17,154 %, 18,15 %, 18,152 %, 18,154 %, 18,155 %, 19,15 %, 19,152 %, 19,154 %, 19,155 %, 19,159 %, 20,13 %, 20,155 %, 20,16 %, 21,157 %, 22,15 %, 22,151 %, 22,152 %, 22,1555 %, 23,15 %, 24,151 %, 24,152 %, 24,155 %, 24,157 %, 24,158 %, 25,15 %, 25,152 %, 25,153 %, 25,156 % ou 26,01 % ;
et/ou, la teneur de Nd étant 15 % ou moins, préférablement 4-13 %, plus préférablement 4,02 %, 5,847 %, 5,84 %, 5,849 %, 5,85 %, 5,851 %, 5,852 %, 5,853 %, 5,854 %, 6,851 %, 6,852 %, 6,853 %, 7,85 %, 8,846 %, 8,847 %, 8,85 %, 8,851 %, 8,852 %, 8,853 %, 9,85 %, 9,851 %, 10,844 %, 10,846 %, 10,849 %, 11,349 %, 11,384 %, 12,341 %, 12,345 %, 12,348 %, 12,35 %, 12,351 %,12,364 %, 12,791 %, 12,802 % ou 12,849 % ;
et/ou, le rapport de la masse de Nd sur la masse totale de R' étant inférieur à 0,5, préférablement 0,1-0,45 ; et/ou, la teneur de R' étant préférablement 29,49-32,53 %, plus préférablement 29,495 %, 29,501 %, 30,003 %, 30,004 %, 30,03 %, 30,441 %, 30,517 %, 30,518 %, 30,957 %, 30,98 %, 31 %, 31,006 %, 31,0065 %, 31,009 %, 31,011 %, 31,012 %, 31,013 %, 31,498 %, 31,504 %, 31,539 %, 31,946 %, 31,972 %, 31,977 %, 31,995 %, 31,999 %, 32 %, 32,001 %, 32,013 %, 32,015 %, 32,021 %, 32,022 %, 32,023 %, 32,024 %, 32,025 %, 32,026 %, 32,027 %, 32,04 %, 32,043 %, 32,437 % ou 32,521 % ;
et/ou, R' comprenant en outre d'autres éléments des terres rares outre Pr et Nd, préférablement Y ;
et/ou, R' comprenant en outre RH, RH étant un élément lourd des terres rares, la sorte de RH préférablement comprenant un ou plusieurs parmi Dy, Tb et Ho, plus préférablement Dy et/ou Tb ; préférablement, le rapport en masse de RH et R' étant préférablement inférieur à 0,253, préférablement 0-0,07, plus préférablement 1,01/32,015, 1,02/30,517, 1,02/32,021, 1,02/32,023, 1,02/32,024, 1,02/32,024, 1,02/32,025, 1,02/32,025, 1,02/32,026, 1,03/32,04, 1,04/32,043, 1,432/32,437, 1,46/30,441, 1,47/31,972, 1,48/31,977, 1,5/32, 1,52/32,521, 1,98/30,98, 1,99/31,995, 1/31,999, 1/32, 2,01/31,011, 2,01/31,013, 2,01/32,013, 2,02/32,022, 2,02/32,027, 2/31 ou 2/31,012 ; la teneur de RH étant préférablement 1-2,5 %, plus préférablement 1 %, 1,01 %, 1,02 %, 1,03 %, 1,04 %, 1,432 %, 1,46 %, 1,47 %, 1,48 %, 1,5 %, 1,52 %, 1,98 %, 1,99 %, 2 %, 2,01 % ou 2,02 % ; lorsque RH comprend Tb, la teneur de Tb étant préférablement 0,5-2 % en poids, plus préférablement 0,7 %, 0,72 %, 0,82 %, 0,9 %, 0,91 %, 1 %, 1,02 %, 1,47 %, 1,48 %, 1,5 %, 1,81 %, 1,88 %, 1,89 %, 1,9 %, 1,91 % ou 2,01 % ; lorsque RH comprend Dy, la teneur de Dy étant préférablement 0,5 % en poids ou moins, plus préférablement 0,1 %, 0,2 %, 0,21 %, 0,3 %, 0,31 % ou 0,312 % ; lorsque RH comprend Ho, la teneur de Ho étant préférablement 0,8-2 %, plus préférablement 0,98 %, 0,99 % ou 1 % ;
et/ou, la teneur de Cu étant 0,34-1,3 %, préférablement 0,341 %, 0,41 %, 0,452 %, 0,47 %, 0,502 %, 0,51 %, 0,52 %, 0,598 %, 0,62 %, 0,648 %, 0,649 %, 0,701 %, 0,702 %, 0,71 %, 0,78 %, 0,79 %, 0,795 %, 0,806 %, 0,81 %, 0,852 %, 0,89 %, 0,901 %, 0,903 %, 0,91 %, 0,92 %, 0,948 %, 1,021 %, 1,05 %, 1,08 %, 1,101 %, 1,103 %, 1,12 %, 1,18 %, 1,19 %, 1,202 % ou 1,21 % ;
et/ou, la teneur de B étant 0,95-1,2 %, préférablement 0,983 %, 0,984 %, 0,985 %, 0,988 %, 0,989 %, 1,02 % ou 1,19 % ;
et/ou, la teneur de Fe étant 64,8-69,2 %, préférablement 64,965 %,65,031 %, 65,095 %, 65,155 %, 65,204 %, 65,36 %, 65,4 %, 65,458 %, 65,525 %, 65,626 %, 65,63 %, 65,686 %, 65,817 %, 65,8395 %, 65,869 %, 65,909 %, 65,963 %, 65,994 %, 65,995 %, 66,039 %, 66,04 %, 66,099 %, 66,157 %, 66,218 %, 66,267 %, 66,364 %, 66,377 %, 66,427 %, 66,437 %, 66,52 %, 66,605 %, 66,671 %, 66,8075 %, 66,81 %, 66,87 %, 67,095 %, 67,12 %, 67,137 %, 67,457 %, 67,578 %, 67,996 %, 68,302 %, 68,556 % ou 69,181 % ;
et/ou, le matériau magnétique de néodyme-fer-bore comprenant en outre Al ; préférablement, la teneur de Al étant 0,5 % ou moins, préférablement 0,03-0,5 % en poids, plus préférablement 0,01 %, 0,02 %, 0,03 %, 0,1 %, 0,102 %, 0,12 %, 0,2 %, 0,21 %, 0,24 %, 0,25 %, 0,29 %, 0,3 %, 0,31 %, 0,38 %, 0,4 %, 0,42 %, 0,45 %, 0,46 % ou 0,48 % ;
et/ou, le matériau magnétique de néodyme-fer-bore comprenant en outre Zr ; préférablement, la teneur de Zr étant 0,05-0,31 % en poids, préférablement 0,1 %, 0,21 %, 0,22 %, 0,25 %, 0,251 %, 0,252 %, 0,261 %, 0,272 %, 0,28 %, 0,281 %, 0,282 %, 0,291 %, 0,3 % ou 0,301 % ;
et/ou, le matériau magnétique de néodyme-fer-bore comprenant en outre Ga ; préférablement, la teneur de Ga étant 0,51 % ou moins, préférablement 0,1-0,51 %, plus préférablement 0,1 %, 0,101 %, 0,102 %, 0,11 %, 0,12 %, 0,152 %, 0,18 %, 0,2 %, 0,202 %, 0,24 %, 0,25 %, 0,251 %, 0,302 %, 0,401 % ou 0,501 % ;
et/ou, le matériau magnétique de néodyme-fer-bore comprenant en outre Co ; préférablement, la teneur de Co étant 0,2-1,5 %, préférablement 0,2 % ou 1 % ; et/ou, le matériau magnétique de néodyme-fer-bore comprenant en outre O ; préférablement, la teneur de O étant 0,13 % ou moins ;
et/ou, le matériau magnétique de néodyme-fer-bore pouvant en outre comprendre un ou plusieurs parmi Zn, Ag, In, Sn, V, Cr, Mo, Ta, Hf et W ; la teneur de Zn étant préférablement 0,02-0,08 %, plus préférablement 0,03 %, 0,04 % ou 0,07 % ; la teneur de Mo étant préférablement 0,01-0,08 %, plus préférablement 0,03 %, 0,06 % ou 0,07 %.

8. Matériau magnétique de néodyme-fer-bore, dans lequel, dans la région triangulaire intragranulaire du matériau magnétique de néodyme-fer-bore, le rapport de la masse totale de Pr et Cu sur la masse totale de chaque élément dans la région triangulaire inter granulaire est Q1 ;
au niveau de la limite de grain du matériau magnétique de néodyme-fer-bore, le rapport de la masse totale de Pr et Cu sur la masse totale de chaque élément au niveau de la limite de grain est Q2 ;
Q1 < Q2, et Q2 ≥ 0,1 ; et
les composants du matériau magnétique de néodyme-fer-bore faisant référence au matériau magnétique de néodyme-fer-bore selon l'une quelconque des revendications 6-7.

9. Application du matériau magnétique de néodyme-fer-bore selon l'une quelconque des revendications 6-8 en tant que composant électronique dans un moteur.
